



US009528071B2

(12) **United States Patent**  
**Hogendoorn et al.**

(10) **Patent No.:** **US 9,528,071 B2**  
(45) **Date of Patent:** **\*Dec. 27, 2016**

(54) **LUBRICATING OIL COMPOSITIONS WITH ENHANCED PISTON CLEANLINESS**

(71) Applicant: **Chevron Oronite Technology B.V.**, Rotterdam (NL)

(72) Inventors: **Richard Hogendoorn**, Prinsenbeek (NL); **Bertus Bernardus Hoogendam**, Rotterdam (NL)

(73) Assignee: **Chevron Oronite Technology B.V.**, Rotterdam (NL)

(\*) Notice: Subject to any disclaimer, the term of this patent is extended or adjusted under 35 U.S.C. 154(b) by 0 days.

This patent is subject to a terminal disclaimer.

(21) Appl. No.: **14/622,079**

(22) Filed: **Feb. 13, 2015**

(65) **Prior Publication Data**

US 2016/0237372 A1 Aug. 18, 2016

(51) **Int. Cl.**

**C10M 161/00** (2006.01)

(52) **U.S. Cl.**

CPC ..... **C10M 161/00** (2013.01)

(58) **Field of Classification Search**

CPC ..... C10M 161/00

See application file for complete search history.

(56) **References Cited**

U.S. PATENT DOCUMENTS

|             |         |                      |
|-------------|---------|----------------------|
| 3,172,892 A | 3/1965  | LeSuer et al.        |
| 3,219,666 A | 11/1965 | Norman et al.        |
| 3,272,746 A | 9/1966  | LeSuer et al.        |
| 3,275,554 A | 9/1966  | Wagenaar             |
| 3,329,658 A | 7/1967  | Fields               |
| 3,361,673 A | 1/1968  | Stuart et al.        |
| 3,368,972 A | 2/1968  | Otto                 |
| 3,405,064 A | 10/1968 | Miller               |
| 3,438,757 A | 4/1969  | Honnen et al.        |
| 3,449,250 A | 6/1969  | Fields               |
| 3,454,555 A | 7/1969  | van der Voort et al. |
| 3,539,663 A | 11/1970 | Pietrusza et al.     |
| 3,565,804 A | 2/1971  | Honnen et al.        |
| 3,574,576 A | 4/1971  | Honnen et al.        |
| 3,649,229 A | 3/1972  | Otto                 |
| 3,666,730 A | 5/1972  | Coleman              |
| 3,909,430 A | 9/1975  | Hotten               |
| 3,912,764 A | 10/1975 | Palmer, Jr.          |
| 3,968,157 A | 7/1976  | Hotten               |
| 4,152,499 A | 5/1979  | Boerzel et al.       |
| 4,157,309 A | 6/1979  | Wilgus et al.        |
| 4,234,435 A | 11/1980 | Meinhardt et al.     |
| 4,605,808 A | 8/1986  | Samson               |

|              |   |         |                   |       |             |
|--------------|---|---------|-------------------|-------|-------------|
| 4,655,949 A  | * | 4/1987  | Landry            | ..... | C07F 1/005  |
| 5,112,507 A  |   | 5/1992  | Harrison          |       | 508/367     |
| 5,137,978 A  |   | 8/1992  | DeGonia et al.    |       |             |
| 5,137,980 A  |   | 8/1992  | DeGonia et al.    |       |             |
| 5,175,225 A  |   | 12/1992 | Ruhe, Jr.         |       |             |
| 5,286,799 A  |   | 2/1994  | Harrison et al.   |       |             |
| 5,319,030 A  |   | 6/1994  | Harrison et al.   |       |             |
| 5,523,417 A  |   | 6/1996  | Blackborow et al. |       |             |
| 5,565,528 A  |   | 10/1996 | Harrison et al.   |       |             |
| 5,616,668 A  |   | 4/1997  | Harrison et al.   |       |             |
| 5,625,004 A  |   | 4/1997  | Harrison et al.   |       |             |
| 5,777,025 A  |   | 7/1998  | Spencer et al.    |       |             |
| 5,792,729 A  |   | 8/1998  | Harrison et al.   |       |             |
| 6,165,235 A  |   | 12/2000 | Kolp et al.       |       |             |
| 6,372,696 B1 |   | 4/2002  | Tipton            |       |             |
| 7,838,470 B2 | * | 11/2010 | Shaw              | ..... | C10M 167/00 |
|              |   |         |                   |       | 508/110     |
| 7,964,543 B2 | * | 6/2011  | Harrison          | ..... | C08F 8/32   |
|              |   |         |                   |       | 508/508     |
| 8,394,747 B2 |   | 3/2013  | Harrison et al.   |       |             |
| 8,455,681 B2 |   | 6/2013  | Harrison et al.   |       |             |
| 8,722,927 B2 |   | 5/2014  | Harrison et al.   |       |             |
| 8,729,297 B2 |   | 5/2014  | Harrison et al.   |       |             |

FOREIGN PATENT DOCUMENTS

|    |           |         |
|----|-----------|---------|
| EP | 542380 A1 | 5/1993  |
| EP | 355895 B1 | 12/1994 |
| EP | 602863 B1 | 5/1997  |

\* cited by examiner

Primary Examiner — Cephia D Toomer

(74) Attorney, Agent, or Firm — Ryan, Mason & Lewis, LLP

(57) **ABSTRACT**

Disclosed herein is lubricating oil composition for providing enhanced piston cleanliness in an internal combustion engine. The lubricating oil composition includes (a) greater than 65 wt. %, based on the total weight of the lubricating oil composition, of a base oil component having a Kv at 100° C. of about 3.5 to about 4.5 cSt; (b) about 3.0 wt. % to about 10 wt. %, based on the total weight of the lubricating oil composition, of at least one Mannich reaction product prepared by the condensation of a polyisobutyl-substituted hydroxyaromatic compound, wherein the polyisobutyl group is derived from polyisobutene containing at least about 70 wt. % methylvinylidene isomer and has a number average molecular weight of from about 400 to about 2,500, an aldehyde, an amino acid or ester derivative thereof, and an alkali metal base; and (c) at least one ashless dispersant other than component (b); wherein the lubricating oil composition has a sulfur content of less than or equal to about 0.30 wt. %, a phosphorus content of less than or equal to about 0.09 wt. %, and a sulfated ash content of less than or equal to about 1.60 wt. % as determined by ASTM D 874, based on the total weight of the lubricating oil composition; and further wherein the lubricating oil composition is a SAE 0W multi-grade lubricating oil composition.

20 Claims, No Drawings

## 1

LUBRICATING OIL COMPOSITIONS WITH  
ENHANCED PISTON CLEANLINESS

## BACKGROUND OF THE INVENTION

## 1. Technical Field

The present invention generally relates to low and medium sulfur, phosphorus, and sulfated ash (low and medium "SAPS") lubricating oil compositions to enhance piston cleanliness in internal combustion engines.

## 2. Description of the Related Art

The viscosity grade of an engine oil is a key feature when selecting a lubricating oil. The lubricating oil is typically chosen according to both the climatic temperatures to which the engine is exposed, and the temperatures and shear conditions under which the engine operates. Thus, the oil must be of sufficiently low viscosity at ambient temperatures to provide adequate lubrication upon cold starting of the engine, and capable of maintaining sufficient viscosity to lubricate the engine when it is under a full operating load.

The Society of Automotive Engineers classification system, SAE J300, defines engine oil grade viscosity specifications. Single grades are designated as SAE 20, 30, 40, 50, and 60 grade, and are defined by a low shear rate kinematic viscosity range at 100° C. (ASTM D445), as well as a minimum high shear rate viscosity at 150° C. (such as ASTM D4683, CEC L-36-A-90, or ASTM D5481). Engine oils designated as SAE 0W through 25W have been classified according to their low temperature cranking viscosities (ASTM D5293), low temperature pumping viscosities (ASTM 4684), and a minimum kinematic viscosity at 100° C.

Multigrade lubricating oils perform over wide temperature ranges. Typically, they are identified by two numbers such as, for example, 5W-30 or 10W-30. The first number in the multigrade designation is associated with a safe cranking temperature (e.g., -20° C.) viscosity requirement for that multigrade oil as measured by a cold cranking simulator (CCS) under high shear rates (ASTM D5293). In general, lubricants that have low CCS viscosities allow the engine to crank more easily at lower temperatures and thus improve engine startability at those ambient temperatures.

The second number in the multigrade designation is associated with a lubricant's viscosity under normal operating temperatures and is measured in terms of the kinematic viscosity (K<sub>v</sub>) at 100° C. (ASTM D445). The high temperature viscosity requirement brackets minimum and maximum kinematic viscosity at 100° C. Viscosity at high temperatures is desirable to prevent engine wear that would result if the lubricant thinned out too much during engine operation. However the lubricant should not be too viscous because excessive viscosity may cause unnecessary viscous drag and work to pump the lubricant which in turn can increase fuel consumption. In general, the lower a lubricants' K<sub>v</sub> 100° C., the better the scores that lubricant achieves in fuel economy tests.

Thus, in order to qualify for a given multigrade oil designation a particular multigrade oil must simultaneously meet both strict low and high temperature viscosity requirements that are set by SAE specifications such as SAE J300.

Merely blending base stocks of different viscosity characteristics may not enable the formulator to meet the low and high temperature viscosity requirements of some multigrade oils. The formulator's primary tool for achieving this goal is an additive conventionally referred to as a viscosity modifier or viscosity index (V.I.) improver. Usually, to reach the minimum high temperature viscosity required, it is neces-

sary to add significant amounts of viscosity modifier. However, the use of an increased amount of viscosity modifier results in increased low temperature lubricant viscosity. The ever increasing need to formulate crankcase lubricants that deliver improved performance in fuel economy tests is driving the industry to engine lubricants in the lower viscosity grades, such as SAE 0W-20, 0W-30, 5W-20 and 5W-30.

Concurrent with the demand for lower viscosity, high fuel economy lubricants, there has been a continued effort to reduce the content of sulfated ash, phosphorus and sulfur in the crankcase lubricant due to both environmental concerns and to insure compatibility with pollution control devices used in combination with modern engines (e.g., three-way catalytic converters and particulate traps). A particularly effective class of antioxidant-antiwear additives available to lubricant formulators is metal salts of dialkyldithiophosphates, particularly zinc salts thereof, commonly referred to as ZDDP. While such additives provide excellent performance, ZDDP contributes each of sulfated ash, phosphorus and sulfur to lubricants.

Catalytic converters typically contain one or more oxidation catalysts, NO<sub>x</sub> storage catalysts, and/or NH<sub>3</sub> reduction catalysts. The catalysts contained therein generally comprise a combination of catalytic metals such as platinum, and metal oxides. Catalytic converters are installed in the exhaust systems, for example, the exhaust pipes of automobiles, to convert the toxic gases to nontoxic gases. The use of catalytic converters is thought to be essential in bucking global warming trends and combating other environmental detriments. The catalysts, however, can be poisoned and rendered less effective, if not useless, as a result of exposure to certain elements or compounds, especially phosphorus compounds such as ZDDP.

Particulate traps are usually installed in the exhaust system, especially in diesel engines, to prevent the carbon black particles or very fine condensate particles or agglomerates thereof (i.e., "diesel soot") from being released into the environment. Aside from polluting air, water, and other elements of the environment, diesel soot is a recognized carcinogen. These traps, however, can be blocked by metallic ash which is the degradation product of metal-containing, lubricating oil additives including common ash-producing detergent additives.

To insure a long service life for the after-treatment devices, it is desirable to identify lubricating oil additives that exert a minimum negative impact on such devices. To this end, OEMs often set various limits for maximum sulfur, phosphorus, and/or sulfated ash levels for "new service fill" and "first fill" lubricants. For example, when used in light-duty passenger-car internal combustion engines, the sulfur levels are typically required to be at or below 0.30 wt. %, the phosphorus levels at or below 0.08 wt. %, and the sulfated ash content at or below 0.8 wt. %. The maximum sulfur, phosphorus and/or sulfated ash levels may differ, however, when the lubricating compositions are used in heavy-duty internal combustion engines. For example, the maximum sulfated ash level may be as high as 1.6 wt. % in those heavy-duty engines. Such lubricating oil compositions are also referred to as "medium SAPS" (i.e., medium sulfated ash, phosphorus, and sulfur). When the maximum sulfated ash level is as high as 1.0 wt. %, the lubricating oil compositions are referred to as "low SAPS" lubricating oil compositions, e.g., for gasoline engines, and "LEDL" (i.e., low emission diesel lubricant) oil compositions for diesel engines.

Various tests have been established and standardized to measure the levels of SAPS in any particular lubricating oil compositions. For example, in Europe, a lubricant meeting the ACEA gasoline and diesel engine low SAPS specification must pass, inter alia, the "CEC L-78-T-99" test, which measures the cleanliness and extent of piston ring sticking after running a Volkswagen turbocharged direct injection automotive diesel engine for an extended time period, cycling alternatively between idle and full power. Similar specifications and testing standards of varied stringencies can also be found in other countries and regions, such as Japan, Canada, and the United States.

Meeting the low SAPS environmental standards however does not eliminate the need to provide adequate lubricant performance. Automobile spark ignition and diesel engines have valve train systems, including valves, cams, and rocker arms, all of which must be lubricated and protected from wear. Further, engine oils must provide sufficient detergency so as to insure engine cleanliness and suppress the production of deposits, which are products of non-combustibles and incomplete, combustibles of hydrocarbon fuels and deterioration of engine oils.

As discussed above, the need to preserve the integrity of catalytic converters has led to the use of less phosphate and phosphorus-containing additives. However, the use of detergents, which are typically metal sulfonate detergents, is often inevitable because of the sustained needs to neutralize the oxidation-derived acids and suspend polar oxidation residues in the lubricant. These detergents, however, contribute to the production of sulfated ash. The amount of ash permitted under most of the current environmental standards can be exceeded by far less metal sulfonate detergent than is necessary to achieve adequate detergency performance. Reducing the levels of detergent overbasing may reduce the level of ash produced, but it also reduces the acid neutralizing capacity of the lubricant composition, potentially leading to acid corrosion of the engine pistons and other parts.

Oil-soluble Mannich condensation products are useful in internal combustion engine lubricating oils. These products generally act as dispersants to disperse sludge, varnish, and lacquer, and prevent the formation of deposits. In general, conventional oil-soluble Mannich condensation products are formed from the reaction of polyisobutyl-substituted phenols with formaldehyde and an amine or a polyamine. For example, U.S. Pat. Nos. 7,964,543; 8,394,747; 8,455,681; 8,722,927 and 8,729,297 disclose that 0.01 wt. % to 10.0 wt. % of a Mannich condensation product formed by combining, under reaction conditions, a polyisobutyl-substituted hydroxyaromatic compound wherein the polyisobutyl group is derived from polyisobutene containing at least 50 weight percent methylvinylidene isomer and having a number average molecular weight in the range of about 400 to about 5000, an aldehyde, an amino acid or ester thereof, and an alkali metal base, can be used in an engine lubricating oil composition. Each of these patents further disclose in the examples that 1 wt. % of the Mannich condensation product was added to a fully formulated SAE grade 5W-30 baseline oil, SAE grade 5W-40 baseline oil and a SAE grade 10W-40 baseline oil.

Thus, there is a need to provide an improved low and medium SAPS lubricating oil composition which is a SAE 0W multi-grade lubricant that can overcome poor fuel economy performance.

#### SUMMARY OF THE INVENTION

In accordance with one embodiment of the present invention, there is provided a lubricating oil composition comprising:

(a) greater than 65 wt. %, based on the total weight of the lubricating oil composition, of a base oil component having a kinematic viscosity (Kv) at 10° C. of about 3.5 to about 4.5 centistokes (cSt);

5 (b) about 3.0 wt. % to about 10 wt. %, based on the total weight of the lubricating oil composition, of at least one Mannich reaction product prepared by the condensation of a polyisobutyl-substituted hydroxyaromatic compound, wherein the polyisobutyl group is derived from polyisobutene containing at least about 70 wt. % methylvinylidene isomer and has a number average molecular weight of from about 400 to about 2,500, an aldehyde, an amino acid or ester derivative thereof, and an alkali metal base; and

10 (c) at least one ashless dispersant other than component

15 (b);

wherein the lubricating oil composition has a sulfur content of less than or equal to about 0.30 wt. %, a phosphorus content of less than or equal to about 0.09 wt. %, and a sulfated ash content of less than or equal to about 1.60 wt. % as determined by ASTM D 874, based on the total weight of the lubricating oil composition; and further wherein the lubricating oil composition is a multigrade lubricating oil composition meeting the specifications for SAE J300 revised November 2007 requirements for a 0W-X multigrade engine oil, wherein X is 20, 30, 40, 50, or 60.

In accordance with a second embodiment of the present invention, there is provided a method for improving the piston cleanliness of an internal combustion engine, the method comprising operating the internal combustion engine with a lubricating oil composition comprising:

(a) greater than 65 wt. %, based on the total weight of the lubricating oil composition, of a base oil component having a Kv at 100° C. of about 3.5 to about 4.5 cSt;

35 (b) about 3.0 wt. % to about 10 wt. %, based on the total weight of the lubricating oil composition, of at least one Mannich reaction product prepared by the condensation of a polyisobutyl-substituted hydroxyaromatic compound, wherein the polyisobutyl group is derived from polyisobutene containing at least about 70 wt. % methylvinylidene isomer and has a number average molecular weight in the range of from about 400 to about 2,500, an aldehyde, an amino acid or ester derivative thereof, and an alkali metal base; and

40 (c) at least one ashless dispersant other than component

45 (b);

wherein the lubricating oil composition has a sulfur content of less than or equal to about 0.30 wt. %, a phosphorus content of less than or equal to about 0.09 wt. %, and a sulfated ash content of less than or equal to about 1.60 wt. % as determined by ASTM D 874, based on the total weight of the lubricating oil composition; and further wherein the lubricating oil composition is a multigrade lubricating oil composition meeting the specifications for SAE J300 revised November 2007 requirements for a 0W-X multigrade engine oil, wherein X is 20, 30, 40, 50, or 60.

In accordance with a third embodiment of the present invention, there is provided a use of a lubricating oil composition comprising:

(a) greater than 65 wt. %, based on the total weight of the lubricating oil composition, of a base oil component having a Kv at 100° C. of about 3.5 to about 4.5 cSt;

60 (b) about 3.0 wt. % to about 10 wt. %, based on the total weight of the lubricating oil composition, of at least one Mannich reaction product prepared by the condensation of a polyisobutyl-substituted hydroxyaromatic compound, wherein the polyisobutyl group is derived from polyisobutene containing at least about 70 wt. % methylvinyl-

nylidene isomer and has a number average molecular weight in the range of from about 400 to about 2,500, an aldehyde, an amino acid or ester derivative thereof, and an alkali metal base; and

(c) at least one ashless dispersant other than component 5  
(b);

wherein the lubricating oil composition has a sulfur content of less than or equal to about 0.30 wt. %, a phosphorus content of less than or equal to about 0.09 wt. %, and a sulfated ash content of less than or equal to about 1.60 wt. % as determined by ASTM D 874, based on the total weight of the lubricating oil composition; and further wherein the lubricating oil composition is a multigrade lubricating oil composition meeting the specifications for SAE J300 revised November 2007 requirements for a 0W-X multigrade engine oil, wherein X is 20, 30, 40, 50, or 60, for improving the piston cleanliness of an internal combustion engine.

Among other factors, the present invention is based on the surprising discovery that the present combination of dispersants can provide enhanced piston cleanliness performance required in modern low and medium SAPS lubricants which are SAE 0W multi-grade lubricants for internal combustion engines. By using the present combination of the dispersants, low and medium SAPS lubricants which are SAE 0W multi-grade lubricants can be prepared which pass a piston cleanliness and ring sticking test thereby resulting in improved fuel economy performance. In addition, it is believed that the present combination of dispersants can further provide seal compatibility in the modern low and medium SAPS lubricants which are SAE 0W multi-grade lubricants for internal combustion engines

#### DETAILED DESCRIPTION OF THE PREFERRED EMBODIMENTS

Prior to discussing the invention in further detail, the following terms will be defined:

##### Definitions

As used herein, the following terms have the following meanings, unless expressly stated to the contrary:

The term "Total Base Number" or "TBN" as used herein refers to the amount of base equivalent to milligrams of KOH in 1 gram of sample. Thus, higher TBN numbers reflect more alkaline products, and therefore a greater alkalinity reserve. The TBN of a sample can be determined by ASTM Test No. D2896-11 issued May 15, 2011 or any other equivalent procedure.

The term "metal" means alkali metals, alkaline earth metals, or mixtures thereof.

The term "alkaline earth metal" refers to calcium, barium, magnesium, and strontium.

The term "alkali metal" refers to lithium, sodium, potassium, rubidium, and cesium.

The term "sulfated ash content" refers to the amount of metal-containing additives (e.g., calcium, magnesium, molybdenum, zinc, etc.) in a lubricating oil composition and is typically measured according to ASTM D874, which is incorporated herein by reference.

The term "Mannich condensation product" as used herein refers to a mixture of products obtained by the condensation reaction of a polyisobutyl-substituted hydroxyaromatic compound with an aldehyde and an amino acid as described herein, to form condensation products having the formulas given below. The formulas given below are provided only as some examples of the Mannich condensation products believed to be of the present invention and are not intended

to exclude other possible Mannich condensation products that may be formed using the methods described herein.



50 wherein R, R<sub>1</sub>, X and W are as defined herein.

The present invention is directed to a lubricating oil composition comprising:

(a) greater than 65 wt. %, based on the total weight of the lubricating oil composition, of a base oil component having a Kv at 100° C. of about 3.5 to about 4.5 cSt;

(b) about 3.0 wt. % to about 10 wt. %, based on the total weight of the lubricating oil composition, of at least one Mannich reaction product prepared by the condensation of a polyisobutyl-substituted hydroxyaromatic compound, wherein the polyisobutyl group is derived from polyisobutene containing at least about 70 wt. % methylvinylidene isomer and has a number average molecular weight in the range of from about 400 to about 2,500, an aldehyde, an amino acid or ester derivative thereof, and an alkali metal base; and

(c) at least one ashless dispersant other than component (b);

wherein the lubricating oil composition has a sulfur content of less than or equal to about 0.30 wt. %, a phosphorus content of less than or equal to about 0.09 wt. %, and a sulfated ash content of less than or equal to about 1.60 wt. %, based on the total weight of the lubricating oil composition; and further wherein the lubricating oil composition is a multigrade lubricating oil composition meeting the specifications for SAE J300 revised November 2007 requirements for a 0W-X multigrade engine oil, wherein X is 20, 30, 40, 50, or 60.

The lubricating oil compositions of the present invention are more desirable from an environmental standpoint than the conventional internal combustion engine lubricating oils that contain higher phosphorous, sulfur and sulfated ash contents. The lubricating oil compositions of the present invention also facilitate longer service lives for the catalytic converters and the particulate traps, while providing the desired piston cleanliness.

In general, the level of sulfur in the lubricating oil compositions of the present invention is less than or equal to about 0.30 wt %, based on the total weight of the lubricating oil composition, e.g., a level of sulfur of about 0.01 wt. % to about 0.30 wt. %. In one embodiment, the level of sulfur in the lubricating oil compositions of the present invention is less than or equal to about 0.20 wt. %, based on the total weight of the lubricating oil composition, e.g., a level of sulfur of about 0.01 wt. % to about 0.20 wt. %. In one embodiment, the level of sulfur in the lubricating oil compositions of the present invention is less than or equal to about 0.10 wt. %, based on the total weight of the lubricating oil composition, e.g., a level of sulfur of about 0.01 wt. % to about 0.10 wt. %.

In one embodiment, the levels of phosphorus in the lubricating oil compositions of the present invention is less than or equal to about 0.09 wt. %, based on the total weight of the lubricating oil composition, e.g., a level of phosphorus of about 0.01 wt. % to about 0.09 wt. %. In one embodiment, the levels of phosphorus in the lubricating oil compositions of the present invention is less than or equal to about 0.08 wt. %, based on the total weight of the lubricating oil composition, e.g., a level of phosphorus of about 0.01 wt. % to about 0.08 wt. %. In one embodiment, the levels of phosphorus in the lubricating oil compositions of the present invention is less than or equal to about 0.07 wt. %, based on the total weight of the lubricating oil composition, e.g., a level of phosphorus of about 0.01 wt. % to about 0.07 wt. %. In one embodiment, the levels of phosphorus in the lubricating oil compositions of the present invention is less than or equal to about 0.05 wt. %, based on the total weight of the lubricating oil composition, e.g., a level of phosphorus of about 0.01 wt. % to about 0.05 wt. %.

In one embodiment, the level of sulfated ash produced by the lubricating oil compositions of the present invention is less than or equal to about 1.60 wt. % as determined by ASTM D 874, e.g., a level of sulfated ash of from about 0.10 to about 1.60 wt. % as determined by ASTM D 874. In one embodiment, the level of sulfated ash produced by the lubricating oil compositions of the present invention is less than or equal to about 1.00 wt. % as determined by ASTM D 874, e.g., a level of sulfated ash of from about 0.10 to about 1.00 wt. % as determined by ASTM D 874. In one embodiment, the level of sulfated ash produced by the lubricating oil compositions of the present invention is less than or equal to about 0.80 wt. % as determined by ASTM D 874, e.g., a level of sulfated ash of from about 0.10 to about 0.80 wt. % as determined by ASTM D 874. In one embodiment, the level of sulfated ash produced by the

lubricating oil compositions of the present invention is less than or equal to about 0.60 wt. % as determined by ASTM D 874, e.g., a level of sulfated ash of from about 0.10 to about 0.60 wt. % as determined by ASTM D 874.

5 The lubricating oil composition of the present invention is a fully formulated, low or medium SAPS multigrade lubricating oil composition meeting the specifications for SAE J300 revised November 2007 requirements for 0W-X multigrade engine oils, wherein X is 20, 30, 40, 50, or 60. In one 10 embodiment, the lubricating oil composition of the present invention is a fully formulated, low or medium SAPS SAE 0W-20 multigrade lubricating oil composition. In one embodiment, the lubricating oil composition of the present invention is a fully formulated, low or medium SAPS SAE 15 0W-30 multigrade lubricating oil composition. In one embodiment, the lubricating oil composition of the present invention is a fully formulated, low or medium SAPS SAE 0W-40 multigrade lubricating oil composition. In one embodiment, the lubricating oil composition of the present 20 invention is a fully formulated, low or medium SAPS SAE 0W-50 multigrade lubricating oil composition. In one embodiment, the lubricating oil composition of the present invention is a fully formulated, low or medium SAPS SAE 0W-60 multigrade lubricating oil composition.

#### 25 Base Oil Component

The lubricating oil composition of the present invention contains greater than 65 wt. %, based on the total weight of the lubricating oil composition, of a base oil component having a Kv at 100° C. of about 3.5 to about 4.5 cSt. In 30 practice, this means that the base oil component is selected from one or more natural oils, synthetic oils or mixtures thereof which meet the foregoing Kv requirements at 100° C. In one embodiment, the lubricating oil composition of the present invention contains at least about 70 wt. %, based on the total weight of the lubricating oil composition, of a base 35 oil component having a Kv at 100° C. of about 3.5 to about 4.5 cSt. In one embodiment, the lubricating oil composition of the present invention contains at least about 75 wt. %, based on the total weight of the lubricating oil composition, of a base oil component having a Kv at 100° C. of about 3.5 to about 4.5 cSt.

In one embodiment, the lubricating oil composition of the present invention contains greater than 65 wt. % and up to about 85 wt. %, based on the total weight of the composition, 45 of a base oil component having a Kv at 100° C. of about 3.5 to about 4.5 cSt. In one embodiment, the lubricating oil composition of the present invention contains from about 70 wt. % to about 85 wt. %, based on the total weight of the lubricating oil composition, of a base oil component having a Kv at 100° C. of about 3.5 to about 4.5 cSt. In one embodiment, the lubricating oil composition of the present invention contains from about 75 wt. % to about 85 wt. %, based on the total weight of the lubricating oil composition, of a base oil component having a Kv at 100° C. of about 3.5 to about 4.5 cSt.

In general, the base oil component having a Kv at 100° C. of about 3.5 to about 4.5 cSt includes at least one mineral oil basestock. In general, the at least one mineral oil basestock used in the base oil composition is selected from any of the 60 natural mineral oils of API Groups I, II, III, IV, V or mixtures of these used in crankcase lubricating oils for spark-ignited and compression-ignited engines. API guidelines define a base stock as a lubricant component that may be manufactured using a variety of different processes.

65 Group I base oils generally refer to a petroleum derived lubricating base oil having a saturates content of less than 90 wt. % (as determined by ASTM D 2007) and/or a total sulfur

content of greater than 300 ppm (as determined by ASTM D 2622, ASTM D 4294, ASTM D 4297 or ASTM D 3120) and has a viscosity index (VI) of greater than or equal to 80 and less than 120 (as determined by ASTM D 2270).

Group II base oils generally refer to a petroleum derived lubricating base oil having a total sulfur content equal to or less than 300 parts per million (ppm) (as determined by ASTM D 2622, ASTM D 4294, ASTM D 4927 or ASTM D 3120), a saturates content equal to or greater than 90 weight percent (as determined by ASTM D 2007), and a viscosity index (VI) of between 80 and 120 (as determined by ASTM D 2270).

Group III base oils generally refer to a petroleum derived lubricating base oil having less than 300 ppm sulfur, a saturates content greater than 90 weight percent, and a VI of 120 or greater. In one embodiment, the Group III base stock contains at least about 95% by weight saturated hydrocarbons. In another embodiment, the Group III base stock contains at least about 99% by weight saturated hydrocarbons. The term "major amount" as used herein is an amount of greater than 50 wt. %, or greater than about 70 wt. %, or from about 80 to about 95 wt. % or from about 85 to about 95 wt. %, based on the total weight of the composition.

Group IV base oils are polyalphaolefins (PAOs).

Group V base oils include all other base oils not included in Group I, II, III, or IV.

In one preferred embodiment, the base oil component having a Kv at 100° C. of about 3.5 to about 4.5 cSt is a Group II or III basestock. In another preferred embodiment, the base oil component having a Kv at 100° C. of about 3.5 to about 4.5 cSt is a Group III basestock.

The lubricating oil composition can contain minor mounts of other base oil components. For example, the lubricating oil composition can contain a minor amount of a base oil derived from natural lubricating oils, synthetic lubricating oils or mixtures thereof.

Suitable base oil includes base stocks obtained by isomerization of synthetic wax and slack wax, as well as hydrocracked base stocks produced by hydrocracking (rather than solvent extracting) the aromatic and polar components of the crude.

Suitable natural oils include mineral lubricating oils such as, for example, liquid petroleum oils, solvent-treated or acid-treated mineral lubricating oils of the paraffinic, naphthenic or mixed paraffinic-naphthenic types, oils derived from coal or shale, animal oils, vegetable oils (e.g., rapeseed oils, castor oils and lard oil), and the like.

Suitable synthetic lubricating oils include, but are not limited to, hydrocarbon oils and halo-substituted hydrocarbon oils such as polymerized and interpolymerized olefins, e.g., polybutylenes, polypropylenes, propylene-isobutylene copolymers, chlorinated polybutylenes, poly(1-hexenes), poly(1-octenes), poly(1-decenes), and the like and mixtures thereof; alkylbenzenes such as dodecylbenzenes, tetradecylbenzenes, dinonylbenzenes, di(2-ethylhexyl)-benzenes, and the like; polyphenyls such as biphenyls, terphenyls, alkylated polyphenyls, and the like; alkylated diphenyl ethers and alkylated diphenyl sulfides and the derivative, analogs and homologs thereof and the like.

Other synthetic lubricating oils include, but are not limited to, oils made by polymerizing olefins of less than 5 carbon atoms such as ethylene, propylene, butylenes, isobutene, pentene, and mixtures thereof. Methods of preparing such polymer oils are well known to those skilled in the art.

Additional synthetic hydrocarbon oils include liquid polymers of alpha olefins having the proper viscosity. Especially

useful synthetic hydrocarbon oils are the hydrogenated liquid oligomers of C<sub>6</sub> to C<sub>12</sub> alpha olefins such as, for example, 1-decene trimer.

Another class of synthetic lubricating oils include, but are not limited to, alkylene oxide polymers, i.e., homopolymers, interpolymers, and derivatives thereof where the terminal hydroxyl groups have been modified by, for example, esterification or etherification. These oils are exemplified by the oils prepared through polymerization of ethylene oxide or propylene oxide, the alkyl and phenyl ethers of these polyoxyalkylene polymers (e.g., methyl poly propylene glycol ether having an average molecular weight of 1,000, diphenyl ether of polyethylene glycol having a molecular weight of 500-1000, diethyl ether of polypropylene glycol having a molecular weight of 1,000-1,500, etc.) or mono- and polycarboxylic esters thereof such as, for example, the acetic esters, mixed C<sub>3</sub>-C<sub>8</sub> fatty acid esters, or the C<sub>13</sub> oxo acid diester of tetraethylene glycol.

Yet another class of synthetic lubricating oils include, but are not limited to, the esters of dicarboxylic acids e.g., phthalic acid, succinic acid, alkyl succinic acids, alkenyl succinic acids, maleic acid, azelaic acid, suberic acid, sebacic acid, fumaric acid, adipic acid, linoleic acid dimer, malonic acids, alkyl malonic acids, alkenyl malonic acids, etc., with a variety of alcohols, e.g., butyl alcohol, hexyl alcohol, dodecyl alcohol, 2-ethylhexyl alcohol, ethylene glycol, diethylene glycol monoether, propylene glycol, etc. Specific examples of these esters include dibutyl adipate, di(2-ethylhexyl)sebacate, di-n-hexyl fumarate, dioctyl sebacate, diisooctyl azelate, diisododecyl azelate, dioctyl phthalate, didecyl phthalate, dieicosyl sebacate, the 2-ethylhexyl diester of linoleic acid dimer, the complex ester formed by reacting one mole of sebacic acid with two moles of tetraethylene glycol and two moles of 2-ethylhexanoic acid and the like.

Esters useful as synthetic oils also include, but are not limited to, those made from carboxylic acids having from about 5 to about 12 carbon atoms with alcohols, e.g., methanol, ethanol, etc., polyols and polyol ethers such as neopentyl glycol, trimethylol propane, pentaerythritol, dipentaerythritol, tripentaerythritol, and the like.

Silicon-based oils such as, for example, polyalkyl-, polyalkoxy- or polyaryloxy-siloxane oils and silicate oils, comprise another useful class of synthetic lubricating oils. Specific examples of these include, but are not limited to, tetraethyl silicate, tetra-isopropyl silicate, tetra-(2-ethylhexyl) silicate, tetra-(4-methyl-hexyl) silicate, tetra-(p-tert-butylphenyl) silicate, hexyl-(4-methyl-2-pentoxyl) disiloxane, poly(methyl)siloxanes, poly(methylphenyl)siloxanes, and the like. Still yet other useful synthetic lubricating oils include, but are not limited to, liquid esters of phosphorous containing acids, e.g., tricresyl phosphate, trioctyl phosphate, diethyl ester of decane phosphonic acid, etc., polymeric tetrahydrofurans and the like.

The lubricating oil may be derived from unrefined, refined and rerefined oils, either natural, synthetic or mixtures of two or more of any of these of the type disclosed hereinabove. Unrefined oils are those obtained directly from a natural or synthetic source (e.g., coal, shale, or tar sands bitumen) without further purification or treatment. Examples of unrefined oils include, but are not limited to, a shale oil obtained directly from retorting operations, a petroleum oil obtained directly from distillation or an ester oil obtained directly from an esterification process, each of which is then used without further treatment. Refined oils are similar to the unrefined oils except they have been further treated in one or more purification steps to improve one or more properties.

11

These purification techniques are known to those of skill in the art and include, for example, solvent extractions, secondary distillation, acid or base extraction, filtration, percolation, hydrotreating, dewaxing, etc. Rerefined oils are obtained by treating used oils in processes similar to those used to obtain refined oils. Such rerefined oils are also known as reclaimed or reprocessed oils and often are additionally processed by techniques directed to removal of spent additives and oil breakdown products.

Lubricating oil base stocks derived from the hydroisomerization of wax may also be used, either alone or in combination with the aforesaid natural and/or synthetic base stocks. Such wax isomerate oil is produced by the hydroisomerization of natural or synthetic waxes or mixtures thereof over a hydroisomerization catalyst.

Natural waxes are typically the slack waxes recovered by the solvent dewaxing of mineral oils; synthetic waxes are typically the wax produced by the Fischer-Tropsch process.

#### Mannich Reaction Product

The lubricating oil composition of the present invention will further contain about 3.0 wt. % to about 10 wt. %, based on the total weight of the lubricating oil composition, of at least one Mannich reaction product prepared by the condensation of a polyisobutyl-substituted hydroxyaromatic compound, wherein the polyisobutyl group is derived from polyisobutene containing at least about 70 wt. % methylvinylidene isomer and has a number average molecular weight in the range of from about 400 to about 2,500, an aldehyde, an amino acid or ester derivative thereof, and an alkali metal base. In general, the principal Mannich condensation product can be represented by the structure of formula I:



wherein each R is independently —CHR'—, R' is a branched or linear alkyl having one carbon atom to about 10 carbon atoms, a cycloalkyl having from about 3 carbon atoms to about 10 carbon atoms, an aryl having from about 6 carbon atoms to about 10 carbon atoms, an alkaryl having from about 7 carbon atoms to about 20 carbon atoms, or an aralkyl having from about 7 carbon atoms to about 20 carbon atoms, R<sub>1</sub> is a polyisobutyl group derived from polyisobutene containing at least about 70 wt. % methylvinylidene isomer and having a number average molecular weight in the range of about 400 to about 2,500;

X is hydrogen, an alkali metal ion or alkyl having one to about 6 carbon atoms;

W is —[CHR"]<sub>m</sub> wherein each R" is independently H, alkyl having one carbon atom to about 15 carbon atoms, or a substituted-alkyl having one carbon atom to about 10 carbon atoms and one or more substituents selected from the group consisting of amino, amido, benzyl, carboxyl, hydroxyl, hydroxyphenyl, imidazolyl, imino, phenyl, sulfide, or thiol; and m is an integer from 1 to 4;

Y is hydrogen, alkyl having one carbon atom to about 10 carbon atoms, —CHR'OH, wherein R' is as defined above, or

12



wherein Y' is —CHR'OH, wherein R' is as defined above; and R, X, and W are as defined above;

Z is hydroxyl, a hydroxyphenyl group of the formula:



wherein R, R<sub>1</sub>, Y', X, and W are as defined above, and n is an integer from 0 to 20, with the proviso that when n=0, Z must be:



wherein R, R<sub>1</sub>, Y', X, and W are as defined above.

In one embodiment, the R<sub>1</sub> polyisobutyl group has a number average molecular weight of about 500 to about 2,500. In one embodiment, the R<sub>1</sub> polyisobutyl group has a number average molecular weight of about 700 to about 1,500. In one embodiment, the R<sub>1</sub> polyisobutyl group has a number average molecular weight of about 700 to about 1,100. In one embodiment, the R<sub>1</sub> polyisobutyl group is derived from polyisobutene containing at least about 70 wt. % methylvinylidene isomer. In one embodiment, the R<sub>1</sub> polyisobutyl group is derived from polyisobutene containing at least about 90 wt. % methylvinylidene isomer.

In the compound of formula I above, X is an alkali metal ion and most preferably a sodium or potassium ion. In another embodiment, in the compound of formula I above, X is alkyl selected from methyl or ethyl.

In one embodiment, R is CH<sub>2</sub>, R<sub>1</sub> is derived from polyisobutene containing at least about 70 wt. % methylvinylidene isomer and a number average molecular weight in the range of about 700 to about 1,100, W is CH<sub>2</sub>, X is sodium ion and n is 0 to 20.

The Mannich condensation products for use in the lubricating oil composition of the present invention can be prepared by combining under reaction conditions a polyisobutyl-substituted hydroxyaromatic compound, wherein the polyisobutyl group has a number average molecular weight in the range of from about 400 to about 2,500, an aldehyde, an amino acid or ester derivative thereof, and an alkali metal base. In one embodiment, Mannich condensation product prepared by the Mannich condensation of:

(a) a polyisobutyl-substituted hydroxyaromatic compound having the formula:



wherein R<sub>1</sub> is a polyisobutyl group derived from polyisobutene containing at least about 70 wt. % methylvinylidene isomer and having a number average molecular weight in the range of about 400 to about 2,500, R<sub>2</sub> is hydrogen or lower alkyl having one carbon atom to about 10 carbon atoms, and R<sub>3</sub> is hydrogen or —OH;

(b) a formaldehyde or an aldehyde having the formula:



wherein R' is branched or linear alkyl having one carbon atom to about 10 carbon atoms, cycloalkyl having from about 3 carbon atoms to about 10 carbon atoms, aryl having from about 6 carbon atoms to about 10 carbon atoms, alkaryl having from about 7 carbon atoms to about 20 carbon atoms, or aralkyl having from about 7 carbon atoms to about 20 carbon atoms;

(c) an amino acid or ester derivative thereof having the formula:



wherein W is —[CHR"]—<sub>m</sub> wherein each R" is independently H, alkyl having one carbon atom to about 15 carbon atoms, or a substituted-alkyl having one carbon atom to about 10 carbon atoms and one or more substituents selected from the group consisting of amino, amido, benzyl, carboxyl, hydroxyl, hydroxyphenyl, imidazolyl, imino, phenyl, sulfide, or thiol; and m is an integer from one to 4, and A is hydrogen or alkyl having one carbon atom to about 6 carbon atoms; and

(d) an alkali metal base.

#### Polyisobutyl-substituted Hydroxyaromatic Compound

A variety of polyisobutyl-substituted hydroxyaromatic compounds can be utilized in the preparation of the Mannich condensation products of this invention. The critical feature is that the polyisobutyl substituent be large enough to impart oil solubility to the finished Mannich condensation product. In general, the number of carbon atoms on the polyisobutyl substituent group that are required to allow for oil solubility of the Mannich condensation product is on the order of about C<sub>20</sub> and higher. This corresponds to a molecular weight in the range of about 400 to about 2,500. It is desirable that the C<sub>20</sub> or higher alkyl substituent on the phenol ring be located in the position para to the OH group on the phenol.

The polyisobutyl-substituted hydroxyaromatic compound is typically a polyisobutyl-substituted phenol wherein the polyisobutyl moiety is derived from polyisobutene containing at least about 70 wt. % methylvinylidene isomer and more preferably the polyisobutyl moiety is derived from

polyisobutene containing at least about 90 wt. % methylvinylidene isomer. The term "polyisobutyl or polyisobutyl substituent" as used herein refers to the polyisobutyl substituent on the hydroxyaromatic ring. The polyisobutyl substituent has a number average molecular weight in the range of about 400 to about 2,500. In one embodiment, the polyisobutyl moiety has a number average molecular weight in the range of about 450 to about 2,500. In one embodiment, the polyisobutyl moiety has a number average molecular weight in the range of about 700 to about 1,500. In one embodiment, the polyisobutyl moiety has a number average molecular weight in the range of about 700 to about 1,100.

In one preferred embodiment, the attachment of the polyisobutyl substituent to the hydroxyaromatic ring is para to the hydroxyl moiety in at least about 60 percent of the total polyisobutyl-substituted phenol molecules. In one embodiment, the attachment of the polyisobutyl substituent to the hydroxyaromatic ring is para to the hydroxyl moiety in at least about 80 percent of the total polyisobutyl-substituted phenol molecules. In one embodiment, the attachment of the polyisobutyl substituent to the hydroxyaromatic ring is para to the hydroxyl moiety on the phenol ring in at least about 90 percent of the total polyisobutyl-substituted phenol molecules.

Di-substituted phenols are also suitable starting materials for the Mannich condensation products of this invention. Di-substituted phenols are suitable provided that they are substituted in such a way that there is an unsubstituted ortho position on the phenol ring. Examples of suitable di-substituted phenols are o-cresol derivatives substituted in the para position with a C<sub>20</sub> or greater polyisobutyl substituent and the like.

In one embodiment, a polyisobutyl-substituted phenol has the following formula:



wherein R<sub>1</sub> is polyisobutyl group derived from polyisobutene containing at least about 70 wt. % methylvinylidene isomer and having a number average molecular weight in the range of about 400 to about 2,500, and Y is hydrogen.

Suitable polyisobutenes may be prepared using boron trifluoride (BF<sub>3</sub>) alkylation catalyst as described in U.S. Pat. Nos. 4,152,499 and 4,605,808, the contents of each of these references being incorporated herein by reference. Commercially available polyisobutenes having a high alkylvinylidene content include Glissopal® 1000, 1300 and 2300, available from BASF.

The preferred polyisobutyl-substituted phenol for use in the preparation of the Mannich condensation products is a mono-substituted phenol, wherein the polyisobutyl substituent is attached at the para-position to the phenol ring. However, other polyisobutyl-substituted phenols that may undergo the Mannich condensation reaction may also be used for preparation of the Mannich condensation products according to the present invention.

## Solvent

Solvents may be employed to facilitate handling and reaction of the polyisobutyl-substituted phenols in the preparation of the Mannich condensation products. Examples of suitable solvents are hydrocarbon compounds such as heptane, benzene, toluene, chlorobenzene, aromatic solvent, neutral oil of lubricating viscosity, paraffins and naphthenes. Examples of other commercially available suitable solvents that are aromatic mixtures include Chevron® Aromatic 100N, neutral oil, Exxon® 150N, neutral oil.

In one embodiment, the Mannich condensation product may be first dissolved in an alkyl-substituted aromatic solvent. Generally, the alkyl substituent on the aromatic solvent has from about 3 carbon atoms to about 15 carbon atoms. In one embodiment, the alkyl substituent on the aromatic solvent has from about 6 carbon atoms to about 12 carbon atoms.

## Aldehydes

Suitable aldehydes for use in forming the Mannich condensation product include formaldehyde or aldehydes having the formula



wherein R' is branched or linear alkyl having from one carbon atom to about 10 carbon atoms, cycloalkyl having from about 3 carbon atoms to about 10 carbon atoms, aryl having from about 6 carbon atoms to about 10 carbon atoms, alkaryl having from about 7 carbon atoms to about 20 carbon atoms, or aralkyl having from about 7 carbon atoms to about 20 carbon atoms.

Representative aldehydes include, but are not limited to, aliphatic aldehydes such as formaldehyde, acetaldehyde, propionaldehyde, butyraldehyde, valeraldehyde, caproaldehyde and heptaldehyde. Aromatic aldehydes are also contemplated for use in the preparation of the Mannich condensation products, such as benzaldehyde and alkylbenzaldehyde, e.g., para-tolualdehyde. Also useful are formaldehyde producing reagents, such as paraformaldehyde and aqueous formaldehyde solutions such as formalin. In one preferred embodiment, an aldehyde for use in the preparation of the Mannich condensation products is formaldehyde or formalin. By formaldehyde is meant all its forms, including gaseous, liquid and solid. Examples of gaseous formaldehyde is the monomer  $\text{CH}_2\text{O}$  and the trimer,  $(\text{CH}_2\text{O})_3$  (trioxane) having the formula given below.



Examples of liquid formaldehyde are the following:

Monomer  $\text{CH}_2\text{O}$  in ethyl ether.

Monomer  $\text{CH}_2\text{O}$  in water which has the formulas  $\text{CH}_2(\text{H}_2\text{O})_2$  (methylene glycol) and  $\text{HO}(-\text{CH}_2\text{O})_n-\text{H}$ .

Monomer  $\text{CH}_2\text{O}$  in methanol which has the formulas  $\text{OHCH}_2\text{OCH}_3$  and  $\text{CH}_3\text{O}(-\text{CH}_2\text{O})_n-\text{H}$ .

Formaldehyde solutions are commercially available in water and various alcohols. In water it is available as a 37%-50% solution. Formalin is a 37% solution in water.

Formaldehyde is also commercially available as linear and cyclic (trioxane) polymers. Linear polymers may be low molecular weight or high molecular weight polymers.

## Amino Acid

Suitable amino acids or ester derivatives thereof for use in forming the Mannich condensation product include amino acids having the formula



10

15

20

25

30

35

40

45

50

55

60

65

wherein W is  $-\text{[CHR''}_m-$ , wherein each R'' is independently H, alkyl having one carbon atom to about 15 carbon atoms, or a substituted-alkyl having one carbon atom to about 10 carbon atoms and one or more substituents selected from the group consisting of amino, amido, benzyl, carboxyl, hydroxyl, hydroxyphenyl, imidazolyl, imino, phenyl, sulfide, or thiol; and m is an integer from one to 4, and A is hydrogen or alkyl having one carbon atom to about 6 carbon atoms. Preferably the alkyl is methyl or ethyl.

In one embodiment, the amino acid is glycine.

The term "amino acid salt" as used herein refers to salts of amino acids having the formula



30

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

TABLE I

| Name       | Formula                                                                                                                                                                                                                                                                                                                                                                                             | Log K <sup>25°C</sup> ionic strength |
|------------|-----------------------------------------------------------------------------------------------------------------------------------------------------------------------------------------------------------------------------------------------------------------------------------------------------------------------------------------------------------------------------------------------------|--------------------------------------|
| Alanine    | $\begin{array}{c} \text{NH}_2 \\   \\ \text{H}_3\text{C}-\text{CH} \\   \\ \text{C}=\text{O} \\   \\ \text{OH} \end{array}$                                                                                                                                                                                                                                                                         | 9.87                                 |
| Arginine   | $\begin{array}{c} \text{H}_2\text{N}-\text{C}=\text{NH}-\text{C}(\text{H}_2)-\text{C}(\text{H}_2)-\text{C}(\text{H}_2)-\text{CH}-\text{C}=\text{O} \\   \quad   \quad   \quad   \quad   \\ \text{NH} \quad \text{H}_2 \quad \text{H}_2 \quad \text{H}_2 \quad \text{NH}_2 \\   \quad   \quad   \quad   \quad   \\ \text{O} \quad \text{O} \quad \text{O} \quad \text{O} \quad \text{O} \end{array}$ | 8.99                                 |
| Asparagine | $\begin{array}{c} \text{H}_2\text{N}-\text{C}=\text{O}-\text{C}(\text{H}_2)-\text{CH}-\text{C}=\text{O} \\   \quad   \\ \text{NH} \quad \text{NH}_2 \\   \quad   \\ \text{O} \quad \text{O} \end{array}$                                                                                                                                                                                            | 8.72 *                               |

17

TABLE I-continued

| Name           | Formula | Log K <sup>25°C</sup> C. ionic strength |
|----------------|---------|-----------------------------------------|
| Aspartic Acid  |         | 10.0                                    |
| Cysteine       |         | 10.77                                   |
| Cystine        |         | 8.80 **                                 |
| Glutamic Acid  |         | 9.95                                    |
| Glutamine      |         | 9.01 *                                  |
| Glycine        |         | 9.78                                    |
| Histidine      |         | 9.08 *                                  |
| Hydroxy-lysine |         |                                         |
| Isoleucine     |         | 9.75                                    |
| Leucine        |         | 9.75                                    |

18

TABLE I-continued

| Name          | Formula | Log K <sup>25°C</sup> C. ionic strength |
|---------------|---------|-----------------------------------------|
| Lysine        |         | 10.69 *                                 |
| Methionine    |         | 9.05                                    |
| Phenylalanine |         | 9.31                                    |
| Serine        |         | 9.21                                    |
| Threonine     |         | 9.10                                    |
| Tyrosine      |         | 10.47                                   |
| Valine        |         | 9.72                                    |

65 \* 0.1 ionic strength.  
 \*\* 20°C. and 0.1 ionic strength.

19

## Alkali Metal Base

Suitable alkali metal base for use in forming the Mannich condensation product include alkali metal hydroxides, alkali metal alkoxides and the like. In one embodiment, the alkali metal base is an alkali metal hydroxide selected from the group consisting of sodium hydroxide, lithium hydroxide or potassium hydroxide.

In one embodiment, the amino acid may be added in the form of its alkali metal ion salt. In one embodiment, the alkali metal ion is a sodium ion or a potassium ion. In one preferred embodiment, the alkali metal ion is a sodium ion.

## General Procedure for Preparation of Mannich Condensation Product

The reaction to form the Mannich condensation products can be carried out batch wise, or in continuous or semi-continuous mode. Normally the pressure for this reaction is atmospheric, but the reaction may be carried out under sub-atmospheric or super atmospheric pressure if desired.

The temperature for this reaction may vary widely. The temperature range for this reaction can vary from about 10° C. to about 200° C., or from about 50° C. to about 150° C., or from about 70° C. to about 130° C.

The reaction may be carried out in the presence of a diluent or a mixture of diluents. It is important to ensure that the reactants come into intimate contact with each other in order for them to react. This is an important consideration because the starting materials for the Mannich condensation products include the relatively non polar polyisobutyl-substituted hydroxyl aromatic compounds and the relatively polar amino acid or ester derivative thereof. It is therefore necessary to find a suitable set of reaction conditions or diluents that will dissolve all the starting materials.

Diluents for this reaction must be capable of dissolving the starting materials of this reaction and allowing the reacting materials to come in contact with each other. Mixtures of diluents can be used for this reaction. Useful diluents for this reaction include water, alcohols, (including methanol, ethanol, isopropanol, 1-propanol, 1-butanol, isobutanol, sec-butanol, butanediol, 2-ethylhexanol, 1-pentanol, 1-hexanol, ethylene glycol, and the like), DMSO, NMP, HMPA, cellosolve, diglyme, various ethers (including diethyl ether, THF, diphenylether, dioxane, and the like), aromatic diluents (including toluene, benzene, o-xylene, m-xylene, p-xylene, mesitylene and the like), esters, alkanes (including pentane, hexane, heptane, octane, and the like), and various natural and synthetic diluent oils (including 100 neutral oils, 150 neutral oils, polyalphaolefins, Fischer-Tropsch derived base oil and the like, and mixtures of these diluents. Mixtures of diluents that form two phases such as methanol and heptane are suitable diluents for this reaction.

The reaction may be carried out by first reacting the hydroxyaromatic compound with the alkali metal base, followed by the addition of the amino acid or ester derivative thereof and the aldehyde, or the amino acid or ester derivative thereof may be reacted with the aldehyde followed by the addition of the hydroxyaromatic compound and the alkali metal base, etc.

It is believed that the reaction of the amino acid, such as glycine, or ester derivative thereof, plus the aldehyde, such as formaldehyde, may produce the intermediate formula

20



which may ultimately form the cyclic formula



30

35

40

45

50

55

60

65

It is believed that these intermediates may react with the hydroxyaromatic compound and the base to form the Mannich condensation products of the present invention.

Alternatively, it is believed that the reaction of the hydroxyaromatic compound with the aldehyde may produce the intermediate formula



It is also believed that this intermediate may react with the amino acid or ester derivative thereof and the base to form the Mannich condensation product of the present invention.

The time of the reaction can vary widely depending on the temperature. The reaction time can vary between about 0.1 hour to about 20 hours, or from about 2 hours to about 10 hours, or from about 3 hours to about 7 hours.

The charge mole ratio (CMR) of the reagents can also vary over a wide range. Table I below gives a listing of the different formulae that can arise if different charge mole ratios are used. At a minimum the oil-soluble Mannich condensation products should preferable contain at least one polyisobutyl-substituted phenol ring and one amino acid group connected by one aldehyde group and one alkali metal. The polyisobutyl-substituted phenol/aldehyde/amino acid/base charge mole ratio for this molecule, also shown in Table 11 below, is 1.0:1.0: 1.0:1.0. Other charge mole ratios are possible and the use of other charge mole ratios can lead to the production of different molecules of different formulae.

TABLE II

| Product | Polyisobutyl-substituted phenol:aldehyde:<br>amino acid:base (CMR) |
|---------|--------------------------------------------------------------------|
|         | 1.0:1.0:1.0:1.0                                                    |
|         | 1.0:2.0:2.0:2.0                                                    |
|         | 2.0:2.0:1.0:1.0                                                    |
|         | 2.0:3.0:2.0:2.0                                                    |
|         | 3.0:4.0:2.0:2.0                                                    |

## Ashless Dispersant

The lubricating oil composition of the present invention will further contain at least one ashless dispersant other than the Mannich reaction product discussed hereinabove. In general, a suitable ashless dispersant can be polyalkylene succinic anhydride ashless dispersants, non-nitrogen containing ashless dispersants and basic nitrogen-containing ashless dispersants. One other such group suitable for use herein as a dispersing agent includes copolymers which contain a carboxylate ester with one or more additional polar function, including amine, amide, imine, imide, hydroxyl, carboxyl, and the like. These products can be prepared by copolymerization of long chain alkyl acrylates or methacrylates with monomers of the above function. Such groups include alkyl methacrylate-vinyl pyrrolidinone copolymers, alkyl methacrylate-dialkylaminoethylmethacrylate copolymers and the like as well as high molecular weight amides and polyamides or esters and polyesters such as tetraethylpentamine, polyvinyl polystearates and other polystearamides.

The polyalkylene succinic anhydride ashless dispersants include polyisobutylene succinic anhydrides (PIBSA). The number average molecular weight of the polyalkylene tail in the polyalkylene succinic anhydrides used herein will be at least about 350 or from about 750 to about 3000 or from about 900 to about 1100.

In one embodiment, a mixture of polyalkylene succinic anhydrides is employed. In this embodiment, the mixture 55 can comprise a low molecular weight polyalkylene succinic anhydride component e.g., a polyalkylene succinic anhydride having a number average molecular weight of from about 350 to about 1000, and a high molecular weight polyalkylene succinic anhydride component, e.g., a polyalkylene succinic anhydride having a number average molecular weight of from about 1000 to about 3000. In one embodiment, both the low and high molecular weight components are polyisobutylene succinic anhydrides. Alternatively, various molecular weights polyalkylene succinic anhydride components can be combined as a dispersant as well as a mixture of the other above referenced dispersants as identified above.

In general, the polyalkylene succinic anhydride is obtained from a reaction product of a polyalkylene such as polyisobutene with maleic anhydride. One can use conventional polyisobutene, or high methylvinylidene polyisobutene in the preparation of such polyalkylene succinic anhydrides. The polyalkylene succinic anhydrides can be prepared using conventional techniques e.g., thermal, chlorination, free radical, acid catalyzed, or any other process in this preparation that is within the purview of one skilled in the art. Examples of suitable polyalkylene succinic anhydrides for use herein are thermal PIBSA (polyisobutylene succinic anhydride) described in U.S. Pat. No. 3,361,673; chlorinated PIBSA described in U.S. Pat. No. 3,172,892; a mixture of thermal and chlorinated PIBSA described in U.S. Pat. No. 3,912,764; high succinic ratio PIBSA described in U.S. Pat. No. 4,234,435; polyPIBSA described in U.S. Pat. Nos. 5,112,507 and 5,175,225; high succinic ratio polyPIBSA described in U.S. Pat. Nos. 5,565,528 and 5,616,668; free radical PIBSA described in U.S. Pat. Nos. 5,286,799, 5,319,030 and 5,625,004; PIBSA made from high methylvinylidene polybutene described in U.S. Pat. Nos. 4,152,499, 5,137,978 and 5,137,980; high succinic ratio PIBSA made from high methylvinylidene polybutene described in European Patent Application Publication No. EP 355 895; terpolymer PIBSA described in U.S. Pat. No. 5,792,729, sulfonic acid PIBSA described in U.S. Pat. No. 5,777,025 and European Patent Application Publication No. EP 542 380; and purified PIBSA described in U.S. Pat. No. 5,523,417 and European Patent Application Publication No. EP 602 863, the contents of each of these references being incorporated herein by reference.

Non-nitrogen containing ashless dispersants include derivatives of polyalkylene succinic anhydrides such as, for example, succinic acids, Group I and/or Group II mono- or di-metal salts of succinic acids, succinate esters formed by the reaction of a polyalkylene succinic anhydride, acid chloride, or other derivatives with an alcohol (e.g., HOR<sup>1</sup> wherein R<sup>1</sup> is an alkyl group of from 1 to 10 carbon atoms) and the like and mixtures thereof.

If desired, the foregoing polyalkylene succinic anhydride ashless dispersants and/or non-nitrogen-containing ashless dispersants can be post-treated with a wide variety of post-treating reagents. For example, the foregoing polyalkylene succinic anhydride and/or non-nitrogen-containing ashless dispersants can be reacted with a cyclic carbonate under conditions sufficient to cause reaction of the cyclic carbonates with a hydroxyl group. The reaction is ordinarily conducted at temperatures ranging from about 0° C. to about 250° C., or from about 100° C. to about 200° C. or from about 50° C. to about 180° C.

The reaction may be conducted neat, wherein the polyalkylene succinic anhydride or non-nitrogen-containing ashless dispersant and the cyclic carbonate are combined in the proper ratio, either alone or in the present of a catalyst (e.g., an acidic, basic or Lewis acid catalyst). Examples of suitable catalysts include, but are not limited to, phosphoric acid, boron trifluoride, alkyl or aryl sulfonic acid, alkali or alkaline carbonate. The same solvents or diluents as described above with respect to the preparing the polyalkylene succinic anhydride may also be used in the cyclic carbonate post-treatment. In one preferred embodiment, a cyclic carbonate for use herein is 1,3-dioxolan-2-one (ethylene carbonate).

Nitrogen-containing basic ashless (metal-free) dispersants contribute to the base number or BN (as can be measured by ASTM D 2896) of a lubricating oil composition to which they are added, without introducing additional

sulfated ash. The basic nitrogen compound used to prepare the colloidal suspensions of the present invention must contain basic nitrogen as measured by ASTM D664 test or D2896. It is preferably oil-soluble. The basic nitrogen compounds are selected from the group consisting of succinimides, polysuccinimides, carboxylic acid amides, hydrocarbyl monoamines, hydrocarbon polyamines, Mannich condensation products of hydrocarbyl-substituted phenols, formaldehyde and polyamines other than the Mannich reaction product discussed herein above, phosphoramides, thiophosphoramides, phosphonamides, dispersant viscosity index improvers, and mixtures thereof. These basic nitrogen-containing compounds are described below (keeping in mind the reservation that each must have at least one basic nitrogen). Any of the nitrogen-containing compositions may be post-treated with, e.g., boron, using procedures well known in the art so long as the compositions continue to contain basic nitrogen.

The succinimide and polysuccinimide ashless dispersants that can be used in the lubricating oil compositions of the present invention are disclosed in numerous references and are well known in the art. Certain fundamental types of succinimides and the related materials encompassed by the term of art "succinimide" are taught in, for example, U.S. Pat. Nos. 3,219,666; 3,172,892; 3,272,746; 4,234,435 and 6,165,235, the contents of which are incorporated by reference herein. Succinic-based dispersants have a wide variety of chemical structures. One class of succinic-based dispersants may be represented by the formula:



wherein each R<sup>1</sup> is independently a hydrocarbyl group, such as a polyolefin-derived group. Typically the hydrocarbyl group is an alkyl group, such as a polyisobutyl group. Alternatively expressed, the R<sup>1</sup> groups can contain about 40 to about 500 carbon atoms, and these atoms may be present in aliphatic forms. R<sup>2</sup> is an alkylene group, commonly an ethylene (C<sub>2</sub>H<sub>4</sub>) group.

The polyalkenes from which the substituent groups are derived are typically homopolymers and interpolymers of polymerizable olefin monomers of 2 to about 16 carbon atoms, and usually 2 to 6 carbon atoms. The amines which are reacted with the succinic acylating agents to form the carboxylic dispersant composition can be monoamines or polyamines.

The term "succinimide" is understood in the art to include many of the amide, imide, and amidine species which may also be formed. The predominant product, however, is a succinimide and this term has been generally accepted as meaning the product of a reaction of an alkenyl substituted succinic acid or anhydride with a nitrogen-containing compound. In one preferred embodiment, a succinimide, because of its commercial availability, are those succinimides prepared from a hydrocarbyl succinic anhydride, wherein the hydrocarbyl group contains from about 24 to about 350 carbon atoms, and an ethylene amine or polyamine, the ethylene amines being especially characterized by ethylene diamine, diethylene triamine, triethylene

tetramine, tetraethylene pentamine, and higher molecular weight polyethylene amines. Particularly preferred are those succinimides prepared from polyisobutetyl succinic anhydride of 70 to 128 carbon atoms and tetraethylene pentamine or higher molecular weight polyethylene amines or mixtures of polyethylene amines such that the average molecular weight of the mixture is about 205 Daltons. In one embodiment of the present invention, an ashless dispersant for use in the lubricating oil composition is a bis-succinimide derived from a polyisobutetyl group having a number average molecular weight of about 700 to about 2300.

Also included within the term "succinimide" are the co-oligomers of a hydrocarbyl succinic acid or anhydride and a polysecondary amine containing at least one tertiary amino nitrogen in addition to two or more secondary amino groups. Ordinarily, this composition has between 1,500 and 50,000 average molecular weight. A typical compound would be that prepared by reacting polyisobutetyl succinic anhydride and ethylene dipiperazine.

If desired, the foregoing succinimides and polysuccinimide ashless dispersants can be post-treated with a wide variety of post-treating reagents, e.g., with a cyclic carbonate, as discussed hereinabove. The resulting post-treated product has one or more nitrogens of the polyamino moiety substituted with a hydroxy hydrocarbyl oxycarbonyl, a hydroxy poly(oxyalkylene) oxycarbonyl, a hydroxyalkylene, hydroxyalkylene poly(oxyalkylene), or mixture thereof.

The foregoing succinimides and polysuccinimides, including the post-treated compositions described above, can also be reacted to form borated dispersants. In addition to boric acid, examples of suitable boron compounds include boron oxides, boron halides and esters of boric acid. Generally, from about 0.1 equivalent to about 1 equivalent of boron compound per equivalent of basic nitrogen or hydroxyl in the compositions of this invention may be employed.

Carboxylic acid amide ashless dispersants are also useful nitrogen-containing ashless dispersants. Typical of such compounds are those disclosed in U.S. Pat. No. 3,405,064, the contents of which are incorporated by reference herein. These compounds are ordinarily prepared by reacting a carboxylic acid or anhydride or ester thereof, having at least 12 to about 350 aliphatic carbon atoms in the principal aliphatic chain and, if desired, having sufficient pendant aliphatic groups to render the molecule oil soluble with an amine or a hydrocarbyl polyamine, such as an ethylene amine, to give a mono or polycarboxylic acid amide. In one embodiment, a carboxylic amide can be prepared from (1) a carboxylic acid of the formula  $R^2COOH$ , where  $R^2$  is  $C_{12-20}$  alkyl or a mixture of this acid with a polyisobutetyl carboxylic acid in which the polyisobutetyl group contains from 72 to 128 carbon atoms and (2) an ethylene polyamine, especially triethylene tetramine or tetraethylene pentamine or mixtures thereof.

Another class of useful nitrogen-containing ashless dispersants are hydrocarbyl monoamines and hydrocarbyl polyamines, preferably of the type disclosed in U.S. Pat. No. 3,574,576, the contents of which are incorporated by reference herein. The hydrocarbyl group, which is preferably alkyl, or olefinic having one or two sites of unsaturation, usually contains from 9 to about 350, or from about 20 to about 200 carbon atoms. In one embodiment, suitable hydrocarbyl polyamines are those which are derived, e.g., by reacting polyisobutetyl chloride and a polyalkylene polyamine, such as an ethylene amine, e.g., ethylene

diamine, diethylene triamine, tetraethylene pentamine, 2-aminoethylpiperazine, 1,3-propylene diamine, 1,2-propylenediamine, and the like.

Yet another class of useful nitrogen-containing ashless dispersants is the Mannich compounds other than the Mannich reaction products discussed hereinabove. These compounds are prepared from a phenol or  $C_{9-200}$  alkylphenol, an aldehyde, such as formaldehyde or formaldehyde precursor such as paraformaldehyde, and an amine compound. The 10 amine may be a mono or polyamine and typical compounds are prepared from an alkylamine, such as methylamine or an ethylene amine, such as, diethylene triamine, or tetraethylene pentamine, and the like. The phenolic material may be sulfurized and preferably is dodecylphenol or a  $C_{80-100}$  alkylphenol. Typical Mannich bases which can be used in 15 this invention are disclosed in U.S. Pat. Nos. 3,539,663, 3,649,229; 3,368,972 and 4,157,309, the contents of which are incorporated by reference herein. U.S. Pat. No. 3,539, 663, the contents of which are incorporated by reference 20 herein, discloses Mannich bases prepared by reacting an alkylphenol having at least 50 carbon atoms, preferably 50 to 200 carbon atoms with formaldehyde and an alkylene polyamine  $HN(ANH)_nH$  where A is a saturated divalent alkyl hydrocarbon of 2 to 6 carbon atoms and n is 1-10 and 25 where the condensation product of said alkylene polyamine may be further reacted with urea or thiourea. The utility of these Mannich bases as starting materials for preparing lubricating oil additives can often be significantly improved by treating the Mannich base using conventional techniques to introduce boron into the compound.

Still yet another class of useful nitrogen-containing ashless dispersants is the phosphoramides and phosphonamides such as those disclosed in U.S. Pat. Nos. 3,909,430 and 3,968,157, the contents of which are incorporated by reference herein. These compounds may be prepared by forming a phosphorus compound having at least one P—N bond. They can be prepared, for example, by reacting phosphorus oxychloride with a hydrocarbyl diol in the presence of a monoamine or by reacting phosphorus oxychloride with a 35 difunctional secondary amine and a mono-functional amine. Thiophosphoramides can be prepared by reacting an unsaturated hydrocarbon compound containing from 2 to 450 or more carbon atoms, such as polyethylene, polyisobutylene, polypropylene, ethylene, 1-hexene, 1,3-hexadiene, isobutylene, 4-methyl-1-pentene, and the like, with phosphorus pentasulfide and a nitrogen-containing compound as defined above, particularly an alkylamine, alkyldiamine, alkylpolyamine, or an alkyleneamine, such as ethylene diamine, diethylenetriamine, triethylenetetramine, tetraethylenepentamine, and the like.

Suitable ashless dispersants may also include amine dispersants, which are reaction products of relatively high molecular weight aliphatic halides and amines, preferably polyalkylene polyamines. Examples of such amine dispersants include those described in, for example, U.S. Pat. Nos. 3,275,554, 3,438,757, 3,454,555 and 3,565,804, the contents of which are incorporated by reference herein.

Suitable ashless dispersants may also be polymeric, which are interpolymers of oil-solubilizing monomers such as 60 decyl methacrylate, vinyl decyl ether and high molecular weight olefins with monomers containing polar substitutes. Examples of polymeric dispersants include those described in, for example, U.S. Pat. Nos. 3,329,658; 3,449,250 and 3,666,730, the contents of which are incorporated by reference herein.

In general, the ashless dispersants will be present in the lubricating oil compositions of the present invention in an

amount ranging from about 0.1 to about 10 wt. %, based on the total weight of the lubricating oil composition. In one embodiment, the ashless dispersants will be present in the lubricating oil compositions of the present invention in an amount ranging from about 1 to about 8 wt. %, based on the total weight of the lubricating oil composition

The lubricating oil compositions of the present invention may also contain other conventional additives that can impart or improve any desirable property of the lubricating oil composition in which these additives are dispersed or dissolved. Any additive known to a person of ordinary skill in the art may be used in the lubricating oil compositions disclosed herein. Some suitable additives have been described in Mortier et al., "Chemistry and Technology of Lubricants", 2nd Edition, London, Springer, (1996); and Leslie R. Rudnick, "Lubricant Additives: Chemistry and Applications", New York, Marcel Dekker (2003), both of which are incorporated herein by reference. For example, the lubricating oil compositions can be blended with anti-oxidants, anti-wear agents, detergents such as metal detergents, rust inhibitors, dehazing agents, demulsifying agents, metal deactivating agents, friction modifiers, pour point depressants, antifoaming agents, co-solvents, package compatibilisers, corrosion-inhibitors, ashless dispersants, dyes, extreme pressure agents and the like and mixtures thereof. A variety of the additives are known and commercially available. These additives, or their analogous compounds, can be employed for the preparation of the lubricating oil compositions of the invention by the usual blending procedures.

In general, the concentration of each of the additives in the lubricating oil composition, when used, may range from about 0.001 wt. % to about 20 wt. %, from about 0.01 wt. % to about 15 wt. %, or from about 0.1 wt. % to about 10 wt. %, based on the total weight of the lubricating oil composition.

The lubricating oil composition of the present invention can contain one or more antioxidants that can reduce or prevent the oxidation of the base oil. Any antioxidant known by a person of ordinary skill in the art may be used in the lubricating oil composition. Non-limiting examples of suitable antioxidants include amine-based antioxidants (e.g., alkyl diphenylamines such as bis-nonylated diphenylamine, bis-octylated diphenylamine, and octylated/butylated diphenylamine, phenyl- $\alpha$ -naphthylamine, alkyl or arylalkyl substituted phenyl- $\alpha$ -naphthylamine, alkylated p-phenylene diamines, tetramethyl-diaminodiphenylamine and the like), phenolic antioxidants (e.g., 2-tert-butylphenol, 4-methyl-2, 6-di-tert-butylphenol, 2,4,6-tri-tert-butylphenol, 2,6-di-tert-butyl-p-cresol, 2,6-di-tert-butylphenol, 4,4'-methylenebis-(2,6-di-tert-butylphenol), 4,4'-thiobis(6-di-tert-butyl-o-cresol) and the like), sulfur-based antioxidants (e.g., dilauryl-3,3'-thiodipropionate, sulfurized phenolic antioxidants and the like), phosphorous-based antioxidants (e.g., phosphites and the like), zinc dithiophosphate, oil-soluble copper compounds and combinations thereof. The amount of the antioxidant may vary from about 0.01 wt. % to about 10 wt. %, from about 0.05 wt. % to about 5 wt. %, or from about 0.1 wt. % to about 3 wt. %, based on the total weight of the lubricating oil composition.

The lubricating oil composition of the present invention can contain a detergent. Metal-containing or ash-forming detergents function as both detergents to reduce or remove deposits and as acid neutralizers or rust inhibitors, thereby reducing wear and corrosion and extending engine life. Detergents generally comprise a polar head with a long hydrophobic tail. The polar head comprises a metal salt of an acidic organic compound. The salts may contain a substan-

tially stoichiometric amount of the metal in which case they are usually described as normal or neutral salts. A large amount of a metal base may be incorporated by reacting excess metal compound (e.g., an oxide or hydroxide) with an acidic gas (e.g., carbon dioxide).

Detergents that may be used include oil-soluble neutral and overbased sulfonates, phenates, sulfurized phenates, thiophosphonates, salicylates, and naphthenates and other oil-soluble carboxylates of a metal, particularly the alkali or alkaline earth metals, e.g., barium, sodium, potassium, lithium, calcium, and magnesium. The most commonly used metals are calcium and magnesium, which may both be present in detergents used in a lubricant, and mixtures of calcium and/or magnesium with sodium.

Commercial products are generally referred to as neutral or overbased. Overbased metal detergents are generally produced by carbonating a mixture of hydrocarbons, detergent acid, for example: sulfonic acid, carboxylate etc., metal oxide or hydroxides (for example calcium oxide or calcium hydroxide) and promoters such as xylene, methanol and water. For example, for preparing an overbased calcium sulfonate, in carbonation, the calcium oxide or hydroxide reacts with the gaseous carbon dioxide to form calcium carbonate. The sulfonic acid is neutralized with an excess of CaO or Ca(OH)<sub>2</sub>, to form the sulfonate.

Overbased detergents may be low overbased, e.g., an overbased salt having a BN below 100. In one embodiment, the BN of a low overbased salt may be from about 5 to about 50. In another embodiment, the BN of a low overbased salt may be from about 10 to about 30. In yet another embodiment, the BN of a low overbased salt may be from about 15 to about 20.

Overbased detergents may be medium overbased, e.g., an overbased salt having a BN from about 100 to about 250. In one embodiment, the BN of a medium overbased salt may be from about 100 to about 200. In another embodiment, the BN of a medium overbased salt may be from about 125 to about 175.

Overbased detergents may be high overbased, e.g., an overbased salt having a BN above 250. In one embodiment, the BN of a high overbased salt may be from about 250 to about 550.

In one embodiment, the detergent can be one or more alkali or alkaline earth metal salts of an alkyl-substituted hydroxyaromatic carboxylic acid. Suitable hydroxyaromatic compounds include mononuclear monohydroxy and polyhydroxy aromatic hydrocarbons having 1 to 4, and preferably 1 to 3, hydroxyl groups. Suitable hydroxyaromatic compounds include phenol, catechol, resorcinol, hydroquinone, pyrogallol, cresol, and the like. The preferred hydroxyaromatic compound is phenol.

The alkyl substituted moiety of the alkali or alkaline earth metal salt of an alkyl-substituted hydroxyaromatic carboxylic acid is derived from an alpha olefin having from about 10 to about 80 carbon atoms. The olefins employed may be linear, isomerized linear, branched or partially branched linear. The olefin may be a mixture of linear olefins, a mixture of isomerized linear olefins, a mixture of branched olefins, a mixture of partially branched linear or a mixture of any of the foregoing.

In one embodiment, the mixture of linear olefins that may be used is a mixture of normal alpha olefins selected from olefins having from about 12 to about 30 carbon atoms per molecule. In one embodiment, the normal alpha olefins are isomerized using at least one of a solid or liquid catalyst.

In another embodiment, the olefins are a branched olefinic propylene oligomer or mixture thereof having from about 20

to about 80 carbon atoms, i.e., branched chain olefins derived from the polymerization of propylene. The olefins may also be substituted with other functional groups, such as hydroxy groups, carboxylic acid groups, heteroatoms, and the like.

In one embodiment, the branched olefinic propylene oligomer or mixtures thereof have from about 20 to about 60 carbon atoms. In one embodiment, the branched olefinic propylene oligomer or mixtures thereof have from about 20 to about 40 carbon atoms.

In one embodiment, at least about 75 mole % (e.g., at least about 80 mole %, at least about 85 mole %, at least about 90 mole %, at least about 95 mole %, or at least about 99 mole %) of the alkyl groups contained within the alkali or alkaline earth metal salt of an alkyl-substituted hydroxyaromatic carboxylic acid such as the alkyl groups of an alkaline earth metal salt of an alkyl-substituted hydroxybenzoic acid detergent are a  $C_{20}$  or higher. In another embodiment, the alkali or alkaline earth metal salt of an alkyl-substituted hydroxyaromatic carboxylic acid is an alkali or alkaline earth metal salt of an alkyl-substituted hydroxybenzoic acid that is derived from an alkyl-substituted hydroxybenzoic acid in which the alkyl groups are the residue of normal alpha-olefins containing at least 75 mole %  $C_{20}$  or higher normal alpha-olefins.

In another embodiment, at least about 50 mole % (e.g., at least about 60 mole %, at least about 70 mole %, at least about 80 mole %, at least about 85 mole %, at least about 90 mole %, at least about 95 mole %, or at least about 99 mole %) of the alkyl groups contained within the alkali or alkaline earth metal salt of an alkyl-substituted hydroxyaromatic carboxylic acid such as the alkyl groups of an alkali or alkaline earth metal salt of an alkyl-substituted hydroxybenzoic acid are about  $C_{14}$  to about  $C_{18}$ .

The resulting alkali or alkaline earth metal salt of an alkyl-substituted hydroxyaromatic carboxylic acid will be a mixture of ortho and para isomers. In one embodiment, the product will contain about 1 to 99% ortho isomer and 99 to 1% para isomer. In another embodiment, the product will contain about 5 to 70% ortho and 95 to 30% para isomer.

The alkali or alkaline earth metal salts of an alkyl-substituted hydroxyaromatic carboxylic acid can be neutral or overbased. Generally, an overbased alkali or alkaline earth metal salt of an alkyl-substituted hydroxyaromatic carboxylic acid is one in which the BN of the alkali or alkaline earth metal salts of an alkyl-substituted hydroxyaromatic carboxylic acid has been increased by a process such as the addition of a base source (e.g., lime) and an acidic overbasing compound (e.g., carbon dioxide).

Sulfonates may be prepared from sulfonic acids which are typically obtained by the sulfonation of alkyl substituted aromatic hydrocarbons such as those obtained from the fractionation of petroleum or by the alkylation of aromatic hydrocarbons. Examples included those obtained by alkyllating benzene, toluene, xylene, naphthalene, diphenyl or their halogen derivatives. The alkylation may be carried out in the presence of a catalyst with alkyllating agents having from about 3 to more than 70 carbon atoms. The alkaryl sulfonates usually contain from about 9 to about 80 or more carbon atoms, preferably from about 16 to about 60 carbon atoms per alkyl substituted aromatic moiety.

The oil soluble sulfonates or alkaryl sulfonic acids may be neutralized with oxides, hydroxides, alkoxides, carbonates, carboxylate, sulfides, hydrosulfides, nitrates, borates and ethers of the metal. The amount of metal compound is chosen having regard to the desired TBN of the final product

but typically ranges from about 100 to about 220 wt. % (preferably at least about 125 wt. %) of that stoichiometrically required.

Metal salts of phenols and sulfurized phenols are prepared by reaction with an appropriate metal compound such as an oxide or hydroxide and neutral or overbased products may be obtained by methods well known in the art. Sulfurized phenols may be prepared by reacting a phenol with sulfur or a sulfur containing compound such as hydrogen sulfide, 5 sulfur monohalide or sulfur dihalide, to form products which are generally mixtures of compounds in which 2 or more phenols are bridged by sulfur containing bridges.

Generally, the amount of the additional detergent can be from about 0.001 wt. % to about 25 wt. %, from about 0.05 15 wt. % to about 20 wt. %, or from about 0.1 wt. % to about 15 wt. %, based on the total weight of the lubricating oil composition.

The lubricating oil composition of the present invention can contain one or more friction modifiers that can lower the 20 friction between moving parts. Any friction modifier known by a person of ordinary skill in the art may be used in the lubricating oil composition. Non-limiting examples of suitable friction modifiers include fatty carboxylic acids; derivatives (e.g., alcohol, esters, borated esters, amides, metal salts and the like) of fatty carboxylic acid; mono-, di- or tri-alkyl 25 substituted phosphoric acids or phosphonic acids; derivatives (e.g., esters, amides, metal salts and the like) of mono-, di- or tri-alkyl substituted phosphoric acids or phosphonic acids; mono-, di- or tri-alkyl substituted amines; mono- or 30 di-alkyl substituted amides and combinations thereof. In some embodiments examples of friction modifiers include, but are not limited to, alkoxylated fatty amines; borated fatty epoxides; fatty phosphites, fatty epoxides, fatty amines, borated alkoxylated fatty amines, metal salts of fatty acids, 35 fatty acid amides, glycerol esters, borated glycerol esters; and fatty imidazolines as disclosed in U.S. Pat. No. 6,372, 696, the contents of which are incorporated by reference herein; friction modifiers obtained from a reaction product of a  $C_4$  to  $C_{75}$ , or a  $C_6$  to  $C_{24}$ , or a  $C_6$  to  $C_{20}$  fatty acid ester 40 and a nitrogen-containing compound selected from the group consisting of ammonia, and an alkanolamine and the like and mixtures thereof. The amount of the friction modifier may vary from about 0.01 wt. % to about 10 wt. %, from about 0.05 wt. % to about 5 wt. %, or from about 0.1 wt. % 45 to about 3 wt. %, based on the total weight of the lubricating oil composition.

The lubricating oil composition of the present invention can contain one or more anti-wear agents that can reduce friction and excessive wear. Any anti-wear agent known by 50 a person of ordinary skill in the art may be used in the lubricating oil composition. Non-limiting examples of suitable anti-wear agents include zinc dithiophosphate, metal (e.g., Pb, Sb, Mo and the like) salts of dithiophosphates, metal (e.g., Zn, Pb, Sb, Mo and the like) salts of dithiocarbamates, metal (e.g., Zn, Pb, Sb and the like) salts of fatty 55 acids, boron compounds, phosphate esters, phosphite esters, amine salts of phosphoric acid esters or thiophosphoric acid esters, reaction products of dicyclopentadiene and thiophosphoric acids and combinations thereof. The amount of the 60 anti-wear agent may vary from about 0.01 wt. % to about 5 wt. %, from about 0.05 wt. % to about 3 wt. %, or from about 0.1 wt. % to about 1 wt. %, based on the total weight of the lubricating oil composition.

In certain embodiments, the anti-wear agent is or 65 comprises a dihydrocarbyl dithiophosphate metal salt, such as zinc dialkyl dithiophosphate compounds. The metal of the dihydrocarbyl dithiophosphate metal salt may be an alkali or

alkaline earth metal, or aluminum, lead, tin, molybdenum, manganese, nickel or copper. In some embodiments, the metal is zinc. In other embodiments, the alkyl group of the dihydrocarbyl dithiophosphate metal salt has from about 3 to about 22 carbon atoms, from about 3 to about 18 carbon atoms, from about 3 to about 12 carbon atoms, or from about 3 to about 8 carbon atoms. In further embodiments, the alkyl group is linear or branched.

The amount of the dihydrocarbyl dithiophosphate metal salt including the zinc dialkyl dithiophosphate salts in the lubricating oil composition disclosed herein is measured by its phosphorus content. In some embodiments, the phosphorus content of the lubricating oil composition disclosed herein is from about 0.01 wt. % to about 0.14 wt., based on the total weight of the lubricating oil composition.

The lubricating oil composition of the present invention can contain one or more foam inhibitors or anti-foam inhibitors that can break up foams in oils. Any foam inhibitor or anti-foam known by a person of ordinary skill in the art may be used in the lubricating oil composition. Non-limiting examples of suitable foam inhibitors or anti-foam inhibitors include silicone oils or polydimethylsiloxanes, fluorosilicones, alkoxyLATED aliphatic acids, polyethers (e.g., polyethylene glycols), branched polyvinyl ethers, alkyl acrylate polymers, alkyl methacrylate polymers, poly-alkoxyamines and combinations thereof. In some embodiments, the foam inhibitors or anti-foam inhibitors comprises glycerol monostearate, polyglycol palmitate, a trialkyl monothiophosphate, an ester of sulfonated ricinoleic acid, benzoylacetone, methyl salicylate, glycerol monooleate, or glycerol dioleate. The amount of the foam inhibitors or anti-foam inhibitors may vary from about 0.001 wt. % to about 5 wt. %, from about 0.05 wt. % to about 3 wt. %, or from about 0.1 wt. % to about 1 wt. %, based on the total weight of the lubricating oil composition.

The lubricating oil composition of the present invention can contain one or more pour point depressants that can lower the pour point of the lubricating oil composition. Any pour point depressant known by a person of ordinary skill in the art may be used in the lubricating oil composition. Non-limiting examples of suitable pour point depressants include polymethacrylates, alkyl acrylate polymers, alkyl methacrylate polymers, di(tetra-paraffin phenol)phthalate, condensates of tetra-paraffin phenol, condensates of a chlorinated paraffin with naphthalene and combinations thereof. In some embodiments, the pour point depressant comprises an ethylene-vinyl acetate copolymer, a condensate of chlorinated paraffin and phenol, polyalkyl styrene or the like. The amount of the pour point depressant may vary from about 0.01 wt. % to about 10 wt. %, from about 0.05 wt. % to about 5 wt. %, or from about 0.1 wt. % to about 3 wt. %, based on the total weight of the lubricating oil composition.

In one embodiment, the lubricating oil composition of the present invention does not contain one or more demulsifiers. In another embodiment, the lubricating oil composition of the present invention can contain one or more demulsifiers that can promote oil-water separation in lubricating oil compositions that are exposed to water or steam. Any demulsifier known by a person of ordinary skill in the art may be used in the lubricating oil composition. Non-limiting examples of suitable demulsifiers include anionic surfactants (e.g., alkyl-naphthalene sulfonates, alkyl benzene sulfonates and the like), nonionic alkoxyLATED alkyl phenol resins, polymers of alkylene oxides (e.g., polyethylene oxide, polypropylene oxide, block copolymers of ethylene oxide, propylene oxide and the like), esters of oil soluble acids, polyoxyethylene sorbitan ester and combinations

thereof. The amount of the demulsifier may vary from about 0.01 wt. % to about 10 wt. %, from about 0.05 wt. % to about 5 wt. %, or from about 0.1 wt. % to about 3 wt. %, based on the total weight of the lubricating oil composition.

5 The lubricating oil composition of the present invention can contain one or more corrosion inhibitors that can reduce corrosion. Any corrosion inhibitor known by a person of ordinary skill in the art may be used in the lubricating oil composition. Non-limiting examples of suitable corrosion inhibitor include half esters or amides of dodecylsuccinic acid, phosphate esters, thiophosphates, alkyl imidazolines, sarcosines and combinations thereof. The amount of the corrosion inhibitor may vary from about 0.01 wt. % to about 5 wt. %, from about 0.05 wt. % to about 3 wt. %, or from about 0.1 wt. % to about 1 wt. %, based on the total weight of the lubricating oil composition.

10 The lubricating oil composition of the present invention can contain one or more extreme pressure (EP) agents that can prevent sliding metal surfaces from seizing under conditions of extreme pressure. Any extreme pressure agent known by a person of ordinary skill in the art may be used in the lubricating oil composition. Generally, the extreme pressure agent is a compound that can combine chemically with a metal to form a surface film that prevents the welding of asperities in opposing metal surfaces under high loads. Non-limiting examples of suitable extreme pressure agents include sulfurized animal or vegetable fats or oils, sulfurized animal or vegetable fatty acid esters, fully or partially esterified esters of trivalent or pentavalent acids of phosphorus, sulfurized olefins, dihydrocarbyl polysulfides, sulfurized Diels-Alder adducts, sulfurized dicyclopentadiene, sulfurized or co-sulfurized mixtures of fatty acid esters and monounsaturated olefins, co-sulfurized blends of fatty acid, 15 fatty acid ester and alpha-olefin, functionally-substituted dihydrocarbyl polysulfides, thia-aldehydes, thia-ketones, epithio compounds, sulfur-containing acetal derivatives, co-sulfurized blends of terpene and acyclic olefins, and polysulfide olefin products, amine salts of phosphoric acid esters or thiophosphoric acid esters and combinations thereof. The amount of the extreme pressure agent may vary from about 0.01 wt. % to about 5 wt. %, from about 0.05 wt. % to about 3 wt. %, or from about 0.1 wt. % to about 1 wt. %, based on the total weight of the lubricating oil composition.

20 The lubricating oil composition of the present invention can contain one or more rust inhibitors that can inhibit the corrosion of ferrous metal surfaces. Any rust inhibitor known by a person of ordinary skill in the art may be used in the lubricating oil composition. Non-limiting examples of suitable rust inhibitors include nonionic polyoxyalkylene agents, e.g., polyoxyethylene lauryl ether, polyoxyethylene higher alcohol ether, polyoxyethylene nonylphenyl ether, polyoxyethylene octylphenyl ether, polyoxyethylene octyl 25 stearyl ether, polyoxyethylene oleyl ether, polyoxyethylene sorbitol monostearate, polyoxyethylene sorbitol monooleate, and polyethylene glycol monooleate; stearic acid and other fatty acids; dicarboxylic acids; metal soaps; fatty acid amine salts; metal salts of heavy sulfonic acid; partial carboxylic acid ester of polyhydric alcohol; phosphoric esters; (short-chain) alketyl succinic acids; partial esters thereof and nitrogen-containing derivatives thereof; synthetic alkylsulfonates, e.g., metal dinonylnaphthalene sulfonates; and the like and mixtures thereof. The amount of the rust inhibitor may vary from about 0.01 wt. % to about 10 wt. %, from about 0.05 wt. % to about 5 wt. %, or from about 0.1 wt. % to about 3 wt. %, based on the total weight of the lubricating oil composition.

The lubricating oil composition of the present invention can contain one or more multifunctional additives. Non-limiting examples of suitable multifunctional additives include sulfurized oxymolybdenum dithiocarbamate, sulfurized oxymolybdenum organophosphorodithioate, oxymolybdenum monoglyceride, oxymolybdenum diethylate amide, amine-molybdenum complex compound, and sulfur-containing molybdenum complex compound.

The lubricating oil composition of the present invention can contain one or more viscosity index improvers. Non-limiting examples of suitable viscosity index improvers include, but are not limited to, olefin copolymers, such as ethylene-propylene copolymers, styrene-isoprene copolymers, hydrated styrene-isoprene copolymers, polybutene, polyisobutylene, polymethacrylates, vinylpyrrolidone and methacrylate copolymers and dispersant type viscosity index improvers. These viscosity modifiers can optionally be grafted with grafting materials such as, for example, maleic anhydride, and the grafted material can be reacted with, for example, amines, amides, nitrogen-containing heterocyclic compounds or alcohol, to form multifunctional viscosity modifiers (dispersant-viscosity modifiers). Other examples of viscosity modifiers include star polymers (e.g., a star polymer comprising isoprene/styrene/isoprene tri-block). Yet other examples of viscosity modifiers include poly alkyl(meth)acrylates of low Brookfield viscosity and high shear stability, functionalized poly alkyl(meth)acrylates with dispersant properties of high Brookfield viscosity and high shear stability, polyisobutylene having a weight average molecular weight ranging from 700 to 2,500 Daltons and mixtures thereof. The amount of the viscosity index improvers may vary from about 0.01 wt. % to about 25 wt. %, from about 0.05 wt. % to about 20 wt. %, or from about 0.3 wt. % to about 15 wt. %, based on the total weight of the lubricating oil composition.

The lubricating oil composition of the present invention can contain one or more metal deactivators. Non-limiting examples of suitable metal deactivators include disalicylidene propylenediamine, triazole derivatives, thiadiazole derivatives, and mercaptobenzimidazoles.

If desired, the at least one Mannich reaction product (b) and/or at least one ashless dispersant (c) may be provided alone or together as an additive package or concentrate in which the at least one Mannich reaction product (b) and/or at least one ashless dispersant (c) and optionally with the foregoing lubricant additives are incorporated into a substantially inert, normally liquid organic diluent such as, for example, mineral oil, naphtha, benzene, toluene or xylene to form an additive concentrate. These concentrates usually contain from about 20% to about 80% by weight of such diluent. Typically, a neutral oil having a viscosity of about 4 to about 8.5 cSt at 100° C. and preferably about 4 to about 6 cSt at 100° C. will be used as the diluent, though synthetic oils, as well as other organic liquids which are compatible with the additives and finished lubricating oil can also be used. The additive package will typically contain one or more of the various additives, referred to above, in the desired amounts and ratios to facilitate direct combination with the requisite amount of the oil of lubricating viscosity.

The lubricating oil composition disclosed herein is used to lubricate an internal combustion engine such as a spark ignition engine, or a compression ignition diesel engine, e.g., a heavy duty diesel engine or a compression ignition diesel engine equipped with at least one of an exhaust gas recirculation (EGR) system; a catalytic converter; and a particulate trap. Such a motor oil composition may be used to lubricate all major moving parts in any reciprocating

internal combustion engine, reciprocating compressors and in steam engines of crankcase design. In automotive applications, the motor oil composition may also be used to cool hot engine parts, keep the engine free of rust and deposits, and seal the rings and valves against leakage of combustion gases.

The primary service classes for a heavy duty diesel engine are light, medium, and heavy heavy-duty diesel engines as disclosed in US 40 CFR 86.090-2. The classification is based on factors such as vehicle gross vehicle weight (GVW), vehicle usage and operating patterns, other vehicle design characteristics, engine horsepower, and other engine design and operating characteristics. The following is a general description of the primary service classes for a heavy duty diesel engine:

(1) Light heavy duty diesel engines usually are non-sleeved and not designed for rebuild; their rated horsepower generally ranges from 70 to 170. Vehicle body types in this group may include any heavy-duty vehicle built for a light-duty truck chassis, van trucks, multi-stop vans, recreational vehicles, and some single axle straight trucks. Typical applications of such engines include personal transportation, light-load commercial hauling and delivery, passenger service, agriculture, and construction. The engines in this group are normally used in vehicles whose GVW is normally less than 19,500 lbs.

(2) Medium heavy duty diesel engines may be sleeved or non-sleeved and may be designed for rebuild; their rated horsepower generally ranges from 170 to 250. Vehicle body types in this group may include school buses, tandem axle straight trucks, city tractors, and a variety of special purpose vehicles such as small dump trucks, and trash compactor trucks. Typical applications of such engines include commercial short haul and intra-city delivery and pickup. The engines in this group are normally used in vehicles whose GVW varies from 19,500 to 33,000 lbs.

(3) Heavy heavy duty diesel engines are sleeved and designed for multiple rebuilds; their rated horsepower generally exceeds 250. Vehicles body types in this group may include tractors, trucks, and buses used in inter-city, long-haul applications. The engines in this group are normally used in vehicles whose GVW exceed 33,000 lbs.

The following non-limiting examples are illustrative of the present invention.

Oil A, and Comparative oils 1 and 2 were prepared and tested for piston cleanliness and tendency to piston ring sticking according to the Volkswagen Turbocharged DI test, a European passenger car diesel engine test (CEC-L-78-T-99), which is part of the ACEA A/B and C specifications promulgated by the European Automobile Manufacturers Association in 2004. This test was used to simulate repeated cycles of high-speed operation followed by idling. A Volkswagen 1.9 liter, inline, four-cylinder turbocharged direct injection automotive diesel engine (VW TDI) was mounted on an engine dynamometer stand. A 54-hour, 2-phased procedure that cycles between 30 minutes of 40° C. oil sump at idle and 150 minutes of 145° C. oil sump at full power (4150 rpm) was carried out without interim oil top-ups. After the procedure, the pistons were rated for carbon and lacquer deposits, as well for groove carbon filling. The piston rings were evaluated for ring sticking. The results are set forth below in Table III. Each of Oil A and Comparative Oils 1 and 2 were formulated to meet the specifications for SAE J300 revised November 2007 requirements for a 0W-20 multi-grade engine oil.

Oil A: A 0W-20 viscosity grade fully formulated lubricating oil composition was prepared comprising 79.23 wt. %

Group III Base oil (4.1 cSt at 100° C.), about 8 wt. % of an ethylene carbonate treated bis-succinimide dispersant, 3.0 wt. % of a Mannich reaction product (a reaction product of a polyisobutyl-substituted phenol (prepared with a 1,000 number average molecular weight polyisobutylene having greater than 70 wt. % methylvinylidene isomer), sodium glycine, and formaldehyde), and typical amounts of detergents, phosphorous antiwear agent, antioxidant, friction modifier, foam inhibitor, viscosity index improver, pour point depressant, and diluent oil. Oil A had a sulfated ash content of about 0.79 wt. %, sulfur content of about 0.18 wt. %, and a phosphorus content of about 0.074 wt. %.

Comparative Oil 1: the formulation of Oil A was substantially duplicated except that Comparative Oil 1 had 79.7 wt. % Group III Base oil (4.1 cSt at 100° C.) and 1.50 wt. % of the Mannich reaction product. Comparative Oil 1 had a sulfated ash content of about 0.82 wt. %, sulfur content of about 0.18 wt. %, and a phosphorus content of about 0.07 wt. %. Comparative Oil 1 was a 0W-20 viscosity grade lubricating oil composition.

Comparative Oil 2: the formulation of Oil A was substantially duplicated except that Comparative Oil 2 had 79.7 wt. % Group III Base oil (4.1 cSt at 100° C.) and 2.25 wt. % of the Mannich reaction product. Comparative Oil 2 had a sulfated ash content of about 0.79 wt. %, sulfur content of about 0.18 wt. %, and a phosphorus content of about 0.074 wt. %. Comparative Oil 2 was a 0W-20 viscosity grade lubricating oil composition.

TABLE III

Test type: VWTDI2; SAE: 0W-20

| Measurements  | Oil A    | Comp. Oil 1 | Comp. Oil 2 |
|---------------|----------|-------------|-------------|
| Inspection    | 54 hours | 54 hours    | 54 hours    |
| PCInC and Avg | 67       | 63          | 61          |
| PCInRL206 Avg | 65       | 65          | 65          |
| AvRS8R4P, ASF | 0        | 0           | 0.31        |
| #RngASF >=2.5 | 0        | 0           | 1           |
| ASFG1RSMAXme  | 0        | 0           | 2.5         |
| ASFG2RSMAXme  | 0        | 0           | 0           |
| Pass/Fail     | Pass VW  | Fail C3     | Fail C3     |

The pass/fail score according to ACEA standards B4, B5, C3, and VW limits are listed in the following Table IV. If the VW 504/507 limits are passed then the remaining specifications are also passed.

TABLE IV

|                        | ACEA A3/B4 limits | ACEA A5/B5 limits | ACEA C3 limits | VW 504/507 limits |
|------------------------|-------------------|-------------------|----------------|-------------------|
| Piston Merit, Avg      | ≥RL206            | (≥RL206)          | (≥RL206)       | (≥RL206 + std)    |
| Ring sticking.         | ≤1.0              | ≤1.0              | ≤1.0           | ≤1.0              |
| Avg. 1st gr, ASF, max. |                   |                   |                |                   |
| Ring sticking.         | ≤1.0              | ≤1.0              | ≤1.0           | ≤1.0              |
| Max. 1st gr, ASF, max. |                   |                   |                |                   |
| Ring sticking.         | ≤0.0              | ≤0.0              | ≤0.0           | ≤0.0              |
| Max. 2nd gr, ASF, max. |                   |                   |                |                   |
| TBN at EOT             | >=6.0             | >=4.0             | Report         |                   |
| TAN at EOT             | Report            | Report            | Report         |                   |

It will be understood that various modifications may be made to the embodiments disclosed herein. Therefore the above description should not be construed as limiting, but

merely as exemplifications of preferred embodiments. For example, the functions described above and implemented as the best mode for operating the present invention are for illustration purposes only. Other arrangements and methods may be implemented by those skilled in the art without departing from the scope and spirit of this invention. Moreover, those skilled in the art will envision other modifications within the scope and spirit of the claims appended hereto.

What is claimed is:

1. A lubricating oil composition comprising:

(a) greater than 65 wt. %, based on the total weight of the lubricating oil composition, of a base oil component having a kinematic viscosity (Kv) at 100° C. of about 3.5 to about 4.5 centistokes (cSt);

(b) about 3.0 wt. % to about 10 wt. %, based on the total weight of the lubricating oil composition, of at least one Mannich reaction product prepared by the condensation of a polyisobutyl-substituted hydroxyaromatic compound, wherein the polyisobutyl group is derived from polyisobutene containing at least about 70 wt. % methylvinylidene isomer and has a number average molecular weight of from about 400 to about 2,500, an aldehyde, an amino acid or ester derivative thereof, and an alkali metal base; and

(c) at least one ashless dispersant other than component (b);

30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8



wherein each R is independently —CHR'—, wherein R' is branched or linear alkyl having one to about 10 carbon atoms, cycloalkyl having from about 3 carbon atoms to about 10 carbon atoms, aryl having from about 6 carbon atoms to about 10 carbon atoms, alkaryl having from about 7 carbon atoms to about 20 carbon atoms, or aralkyl having from about 7 carbon atoms to about 20 carbon atoms, R<sub>1</sub> is a polyisobutyl group derived from polyisobutene containing at least about 70 wt. % methylvinylidene isomer and having a number average molecular weight in the range of about 400 to about 2,500;

X is hydrogen, an alkali metal ion, or alkyl having one carbon atom to about 6 carbon atoms;

W is —[CHR"]<sub>m</sub> wherein each R" is independently H, alkyl having one carbon atom to about 15 carbon atoms, or a substituted-alkyl having one carbon atom to about 10 carbon atoms and one or more substituents selected from the group consisting of amino, amido, benzyl, carboxyl, hydroxyl, hydroxyphenyl, imidazolyl, imino, phenyl, sulfide, or thiol; and m is an integer from one to 4;

Y is hydrogen, alkyl having one carbon atom to about 10 carbon atoms, —CHR'OH, wherein R' is as defined above,

or



wherein Y' is —CHR'OH, wherein R' is as defined above; and R, X, and W are as defined above;

Z is hydroxyl, a hydroxyphenyl group of the formula



wherein R, R<sub>1</sub>, Y', X, and W are as defined above,

and n is an integer from 0 to 20, with the proviso that when n=0, Z must be:



wherein R, R<sub>1</sub>, Y', X, and W are as defined above.

10 15 16. The lubricating oil composition of claim 1, wherein the at least one ashless dispersant is selected from the group consisting of a polyalkylene succinic anhydride ashless dispersant, a non-nitrogen containing ashless dispersant and a basic nitrogen-containing ashless dispersant.

20 25 17. The lubricating oil composition of claim 1, wherein the at least one ashless dispersant is present in an amount ranging from about 0.1 wt. % to about 10 wt. %, based on the total weight of the lubricating oil composition.

25 30 18. The lubricating oil composition of claim 1, further comprising one or more lubricating oil additives selected from the group consisting of an antioxidant, detergent, rust inhibitor, dehazing agent, demulsifying agent, metal deactivating agent, friction modifier, antiwear agent, pour point depressant, antifoaming agent, co-solvent, package compatibiliser, corrosion-inhibitor, dye, extreme pressure agent and mixtures thereof.

35 36 19. The lubricating oil composition of claim 1, which is a heavy duty diesel engine lubricating oil composition.

40 41 20. A method for improving the piston cleanliness of an internal combustion engine, the method comprising operating the internal combustion engine with a lubricating oil composition comprising:

45 46 21. (a) greater than 65 wt. %, based on the total weight of the lubricating oil composition, of a base oil component having a Kv at 100° C. of about 3.5 to about 4.5 cSt; (b) about 3.0 wt. % to about 10 wt. %, based on the total weight of the lubricating oil composition, of at least one Mannich reaction product prepared by the condensation of a polyisobutyl-substituted hydroxyaromatic compound, wherein the polyisobutyl group is derived from polyisobutene containing at least about 70 wt. % methylvinylidene isomer and has a number average molecular weight in the range of from about 400 to about 2,500, an aldehyde, an amino acid or ester derivative thereof and an alkali metal base; and

50 51 22. (c) at least one ashless dispersant other than component (b);

55 56 23. wherein the lubricating oil composition has a sulfur content of less than or equal to about 0.30 wt. %, a phosphorus content of less than or equal to about 0.09 wt. %, and a sulfated ash content of less than or equal to about 1.60 wt. % as determined by ASTM D 874, based on the total weight of the lubricating oil composition; and further wherein the 60 61 lubricating oil composition is a multigrade lubricating oil composition meeting the specifications for SAE J300 revised November 2007 requirements for a 0W-X multi-grade engine oil, wherein X is 20, 30, 40, 50, or 60.

65 66 24. The method of claim 14, wherein the base oil component is a Group III base oil.

67 68 25. The method of claim 14, wherein the at least one Mannich reaction product is of the formula

39



wherein each R is independently  $-\text{CHR}'-$ , wherein R' is branched or linear alkyl having one to about 10 carbon atoms, cycloalkyl having from about 3 carbon atoms to about 10 carbon atoms, aryl having from about 6 carbon atoms to about 10 carbon atoms, alkaryl having from about 7 carbon atoms to about 20 carbon atoms, or aralkyl having from about 7 carbon atoms to about 20 carbon atoms, R<sub>1</sub> is a polyisobutyl group derived from polyisobutene containing at least about 70 wt. % methylvinylidene isomer and having a number average molecular weight in the range of about 400 to about 2,500;

X is hydrogen, an alkali metal ion, or alkyl having one carbon atom to about 6 carbon atoms;

W is  $-\text{[CHR'']}_m-$  wherein each R'' is independently H, alkyl having one carbon atom to about 15 carbon atoms, or a substituted-alkyl having one carbon atom to about 10 carbon atoms and one or more substituents selected from the group consisting of amino, amido, benzyl, carboxyl, hydroxyl, hydroxyphenyl, imidazolyl, imino, phenyl, sulfide, or thiol; and m is an integer from one to 4;

Y is hydrogen, alkyl having one carbon atom to about 10 carbon atoms,  $-\text{CHR}'\text{OH}$ , wherein R' is as defined above,

or



wherein Y' is  $-\text{CHR}'\text{OH}$ , wherein R' is as defined above; and R, X, and W are as defined above;

US 9,528,071 B2

40

Z is hydroxyl, a hydroxyphenyl group of the formula



wherein R, R<sub>1</sub>, Y', X, and W are as defined above, and n is an integer from 0 to 20, with the proviso that when n=0, Z must be:



wherein R, R<sub>1</sub>, Y', X, and W are as defined above.

17. The method of claim 14, wherein the at least one ashless dispersant is selected from the group consisting of a polyalkylene succinic anhydride ashless dispersant, a non-nitrogen containing ashless dispersant and a basic nitrogen-containing ashless dispersant.

18. The method of claim 14, wherein the at least one ashless dispersant is present in the lubricating oil composition in an amount ranging from about 0.1 wt. % to about 10 wt. %, based on the total weight of the lubricating oil composition.

19. The method of claim 14, wherein the lubricating oil composition further comprises one or more lubricating oil additives selected from the group consisting of an antioxidant, detergent, rust inhibitor, dehazing agent, demulsifying agent, metal deactivating agent, friction modifier, antiwear agent, pour point depressant, antifoaming agent, co-solvent, package compatibiliser, corrosion-inhibitor, dye, extreme pressure agent and mixtures thereof.

20. The method of claim 14, wherein the internal combustion engine is a heavy duty diesel engine.

\* \* \* \* \*